# EUROPEAN PATENT SPECIFICATION

(11) **EP 0 423 727 B1**
(45) Date of publication and mention of the grant of the patent: **11.01.1995**
(21) Application number: 90119841.6
(22) Date of filing: 16.10.1990
(51) Int. Cl.: G03C 7/305, G03C 7/333

(54) **Silver halide color photographic material containing colored coupler**
Farbfotografisches Silberhalogenidmaterial, das einen gefärbten Kuppler enthält
Matériau photographique couleur à l'halogénure d'argent contenant un coupleur coloré

(30) Priority: 16.10.1989 JP 268574/89; 29.12.1989 JP 343586/89; 29.12.1989 JP 343587/89; 20.02.1990 JP 39297/90
(43) Date of publication of application: 24.04.1991
(73) Proprietor: FUJI PHOTO FILM CO., LTD., Kanagawa (JP)
(72) Inventor: Kobayashi, Hidetoshi, c/o Fuji Photo Film Co. Ltd., Minami Ashigara-shi, Kanagawa (JP); Ohkawa, Atsuhiro, c/o Fuji Photo Film Co., Ltd., Minami Ashigara-shi, Kanagawa (JP); Mihayashi, Keiji, c/o Fuji Photo Film Co., Ltd., Minami Ashigara-shi, Kanagawa (JP); Kamino, Takayoshi, c/o Fuji Photo Film Co., Ltd., Minami Ashigara-shi, Kanagawa (JP); Motoki, Masuzi, c/o Fuji Photo Film Co., Ltd., Minami Ashigara-shi, Kanagawa (JP)
(74) Representative: Hansen, Bernd, Dr. Dipl.-Chem.

(56) References cited:
- EP-A- 0 161 626
- PATENT ABSTRACTS OF JAPAN vol. 13, no. 138 (P-852)(3486) 06 April 1989, & JP-A-63 304242 (FUJI PHOTO FILM) 12 December 1988,
- PATENT ABSTRACTS OF JAPAN vol. 8, no. 151 (P-286)(1588) 13 July 1984, & JP-A-59 48764 (FUJI PHOTO FILM) 21 March 1984,

## Description

This invention relates to a processing method for color photographic material having improved color reproducibility and more particularly for a silver halide color photographic material containing a colored coupler for color correction, which can release a water-soluble pyridone azo dye.

It is well known that when silver halide color photographic materials are developed, the oxidants of oxidized aromatic primary amine developing agents are coupled with couplers to form dyes such as indophenol, indoaniline, indamine, azomethine, phenoxazine, phenazine and the like, whereby dye images are formed.

Usually, color reproduction by subtractive color photography is conducted in this system. Silver halide emulsions selectively sensitive to blue light, green light and red light, respectively, are used in combination with yellow, magenta, and cyan dye-forming couplers which are complementary color to the light.

The thus-formed dye images do not have always ideal spectral absorption characteristics and often absorb light beyond the primary wavelength range, because absorption is spread, the absorption curve is extended or there is secondary absorption. For example, a cyan dye image should absorb only red light, but generally absorbs some undesirable green light and blue light. A magenta dye image should absorb only green light, but absorbs some undesirable blue light and red light.

It is known to use a masking method using colored couplers to correct the undesirable absorption of a developed color image. For example, this method is described in PSA Journal, Vol. 13, page 94 (1947).

To correct the unnecessary absorption of dye images formed from cyan couplers or magenta couplers, there have been proposed colored couplers described in U.S. Patents 3,583,971, 3,996,055, 4,004,929 and 4,138,258, U.K. Patents 1,324,287 and 1,523,937, JP-A-61-221748 (the term "JP-A" as used herein means an "unexamined published Japanese patent application") and JP-A-61-273543. Magenta colored cyan couplers are used to correct the undesirable absorption mainly of the cyan dye image in the green light region.

The color correction effect of the colored couplers can be achieved when couplers containing a dye structure give developed color images by coupling with oxidized aromatic primary amine developing agents and at the same time the original dye structure is decomposed or flows into developing solutions whereby its absorption is lost (decolorization).

As such decolorizable dye structures, there have been proposed various structures such as azo dyes, azomethine dyes, benzylidene dyes, oxonol dyes, merocyanine dyes, cyanine dyes, styryl dyes, hemioxonol dyes, anthraquinone dyes and xanthene dyes.

However, known yellow colored couplers (e.g., yellow colored cyan couplers) for correcting the unnecessary absorption of cyan dye images in the blue light region are few, including those described in JP-A-61-221748. Decolorizable dye structures are limited to arylene azo dyes and styryl dyes. The characteristics required for the yellow colored couplers are that the molecular extinction coefficient is high; the spectral absorption characteristics are close to the undesired absorption of the dye images of couplers used in combination in the blue light region; and the yellow dye images have high fastness to heat and light. However, the above-described yellow colored couplers are not always fully satisfactory with respect to their performance. For example, they have the disadvantages that molecular extinction coefficient is low, the hue is orange to reddish, or the fastness of the yellow dye images is inferior.

JP-A-63 30 42 42 describes a silver halide color photographic material comprising a layer containing a color coupler capable of releasing a water-soluble compound comprising a 6-hydroxy-2-pyridone-5-azo group. The material described in said document is subjected to a dry processing method.

The object of the invention is to provide a processing method for a silver halide colour photographic material containing a colour coupler having excellent spectral characteristics, having a high molecular extinction coeffecient, resulting in a dye image having high fastness and having improved color reproduceability.

The invention is directed to a processing method comprising subjecting an image-wise exposed silver halide color photographic material comprising a support having thereon at least one light-sensitive silver halide emulsion layer and at least one colored coupler capable of releasing a water-soluble compound comprising a 6-hydroxy-2-pyridone-5-azo group by a coupling reaction with an oxidized aromatic primary amine developing agent to a wet color developing step and a step which uses a bath having bleaching ability.

The colored couplers according to the present invention are illustrated in greater detail.

Preferably, the colored couplers of the present invention are represented by formula (I):

In formula (I), Cp represents a group (a coupler moiety) where the bond between Cp and -(T)_{ℓ} is cleaved by the coupling reaction of the coupler with an oxidized aromatic primary amine developing agent; T represents a timing group; ℓ is 0 or 1; X represents a divalent linking group which is bonded to (T)_{ℓ} through N, O or S; Y represents an arylene group or a divalent heterocyclic group; R₁ and R₂, which may be the same or different each represents a hydrogen atom, a carboxyl group, a sulfo group, a cyano group, an alkyl group, a cycloalkyl group, an aryl group, a heterocyclic group, a carbamoyl group, a sulfamoyl group, a carbonamido group, a sulfonamido group or an alkylsulfonyl group; and R₃ represents a hydrogen atom, an alkyl group, a cycloalkyl group, an aryl group or a heterocyclic group, provided that at least one of R₁, R₂ and R₃ contains a water-solubilizing group (e.g., hydroxyl, carboxyl, sulfo, amino, ammonium, phosphono, phosphino, hydroxysulfonyloxy).

As used herein the group represented by
exists in the following tautomeric form, and all such tautomeric forms of the compounds of formula (I) are included within the scope of the present invention.

The compounds represented by formula (I) are illustrated in more detail.

Conventional groups can be used as the coupler moiety represented by Cp, including yellow coupler moieties (e.g., open chain ketomethylene type couplers moieties), magenta coupler moieties (e.g., 5-pyrazolone type, pyrazoloimidazole type and pyrazolotriazole type coupler moieties), cyan coupler moieties (e.g., phenol type and naphthol type coupler moieties) and non-color forming coupler moieties (e.g., indanone type and acetophenone type coupler moieties). Heterocyclic type coupler moieties described in U.S. Patent 4,315,070, 4,183,752, 3,961,959 or 4,171,223 can be used.

Preferred examples of Cp include coupler moieties represented by formulas (Cp-1), (Cp-2), (Cp-3), (Cp-4), (Cp-5), (Cp-6), (Cp-7), (Cp-8), (Cp-9), and (Cp-10).

These coupler moieties are preferred, because they have a high coupling rate.

In the above formulas, the free bonds at the coupling positions represent the bonding positions of the groups which are eliminated by coupling.

When R₅₁, R₅₂, R₅₃, R₅₄, R₅₅, R₅₆, R₅₇, R₅₈, R₅₉, R₆₀, R₆₁, R₆₂, or R₆₃ in the above formulas contains a nondiffusible group, the total number of carbon atoms in the group is 8 to 40, preferably 10 to 30. In other cases, the total number of carbon atoms is preferably not more than 15. When the couplers are bis type, telomer type or polymer type, any one of the above substituent groups is a bivalent group bonded to a repeating unit. In this case, the total numbers of carbon atoms may be beyond the above range.

R₅₁ to R₆₃, d and e are now illustrated in detail.

Hereinafter, R₄₁ represents an aliphatic group, an aromatic group or a heterocyclic group; R₄₂ represents an aromatic group or a heterocyclic group; and R₄₃, R₄₄, and R₄₅, which may be the same or different, each represents a hydrogen atom, an aliphatic group, an aromatic group or a heterocyclic group.

R₅₁ has the same meaning as R₄₁; R₅₂ and R₅₃ each has the same meaning as R₄₂; R₅₄ represents R₄₁,
R₄₁S-, R₄₃O-,
N≡C-; R₅₅ has the same meaning as R₄₁; R₅₆ and R₅₇ each repersents R₄₃, R₄₁S-, R₄₃O-,
R₅₈ has the same meaning as R₄₁; R₅₉ represents R₄₁,
R₄₁O-, R₄₁S-, a halogen atom or
d is 0 or an integer of from 1 to 3 and when d is 2 or 3, plural R₅₉ groups may be the same or different, or each R₅₉ is a divalent group and these divalent groups may be linked to form a ring structure. Typical examples of the divalent groups which form a ring structure include the following groups.
wherein f is O or an integer of 1 to 4 and g is 0, 1 or 2.

R₆₀ has the same meaning as R₄₁; R₆₁ has the same meaning as R₄₁; R₆₂ represents R₄₁, R₄₁CONH-, R₄₁OCONH-, R₄₁SO₂NH-,
R₄₃O-, R₄₁S-, a halogen atom or
R₆₃ represents R₄₁,
R₄₁SO₂-, R₄₃OCO-, R₄₃O-SO₂-, a halogen atom, a nitro group, a cyano group or R₄₃CO-; and e is 0 or an integer of 1 to 4. When two or more R₆₂ or R₆₃ groups are present, they may be the same or different.

In the present invention groups are defined as follows, unless otherwise defined.

The aliphatic group is a saturated or unsaturated linear or cyclic straight-chain or branched chain, substituted or unsubstituted aliphatic hydrocarbon group having 1 to 32 carbon atoms, preferably 1 to 22 carbon atoms. Typical examples thereof include a methyl group, ethyl group, propyl group, isopropyl group, butyl group, t-butyl group, i-butyl group, t-amyl group, hexyl group, cyclohexyl group, 2-ethylhexyl group, octyl group, 1,1,3,3-tetramethylbutyl group, decyl group, dodecyl group, hexadecyl group and octadecyl group. The aromatic group is a substituted or unsubstituted phenyl or naphthyl group having 6 to 20 carbon atoms. The heterocyclic group is preferably a 3-membered to 8-membered a substituted or unsubstituted heterocyclic group having 1 to 20 carbon atoms, preferably 1 to 7 carbon atoms wherein the hetero-atom is selected from a nitrogen, oxygen and sulfur atom. Typical examples of the heterocyclic group include a 2-pyridyl group, 2-thienyl group, 2-furyl group, 1-imidazolyl group, 1-indolyl group, phthalimido group, 1,3,4-thiadiazole-2-yl group, 2-quinolyl group, 2,4-dioxo-1,3-imidazolidine-5-yl group, 2,4-dioxo-1,3-imidazolidine-3-yl group, succinimido group, 1,2,4-triazole-2-yl group and 1-pyrazolyl group.

The above-described aliphatic hydrocarbon group, aromatic group and heterocyclic group may optionally have one or more substituent groups. Typical examples of such substituent groups include a halogen atom, R₄₇O-, R₄₆S-,
R₄₆SO₂-, R₄₇OCO-,
R₄₆,
R₄₆COO-, R₄₇OSO₂-, a cyano group and a nitro group, wherein R₄₆ represents an aliphatic group, an aromatic group or a heterocyclic group and R₄₇, R₄₈ and R₄₉ each represents an aliphatic group, an aromatic group, a heterocyclic group or a hydrogen atom. The aliphatic group, the aromatic group and the heterocyclic group have the same meanings as those described above.

Preferred examples of R₅₁ to R₆₃ and d and e are as follows.

Preferably, R₅₁ is an aliphatic group or an aromatic group. Preferably, R₅₂, R₅₃ and R₅₅ are each an aromatic group. R₅₄ is preferably R₄₁CONH- or
R₅₆ and R₅₇ are each preferably an aliphatic group, R₄₁O- or R₄₁S-; and R₅₈ is preferably an aliphatic group or an aromatic group. In formula (Cp-6), R₅₉ is preferably a chlorine atom, an aliphatic group or ₄₁CONH-; d is preferably 1 or 2; and R₆₀ is preferably an aromatic group. In formula (Cp-7), R₅₉ is preferably R₄₁CONH-; d is preferably 1; and R₆₁ is preferably an aliphatic group or an aromatic group. In formula (Cp-8), e is preferably 0 or 1; R₆₂ is preferably R₄₁OCONH-, R₄₁CONH- or R₄₁SO₂NH- and these groups are preferably attached to the 5-position of the naphthol ring. In formula (Cp-9), R₆₃ is preferably R₄₁CONH-, R₄₁SO₂NH-,
R₄₁SO₂-,
a nitro group or a cyano group. In formula (Cp-10), R₆₃ is preferably
R₄₃OCO- or a R₄₃CO-.

Examples of R₅₁ to R₆₃ are as follows.

Examples of R₅₁ include a t-butyl group, 4-methoxyphenyl group, phenyl group, 3-{2-(2,4-di-t-amylphenoxy)butaneamido}phenyl group and methyl group. Typical examples of R₅₂ and R₅₃ include 2-chloro-5-dodecyloxycarbonylphenyl group, 2-chloro-5-hexadecylsulfonamidophenyl group, 2-chloro-5-tetradecaneamidophenyl group, 2-chloro-5-{4-(2,4-di-t-amylphenoxy)butaneamido}phenyl group, 2-chloro-5-{2-(2,4-di-t-amylphenoxy)butaneamido}phenyl group, 2-methoxyphenyl group, 2-methoxy-5-tetradecyloxycarbonylphenyl group, 2-chloro-5-(1-ethoxycarbonylethoxycarbonyl)phenyl group, 2-pyridyl group, 2-chloro-5-octyloxycarbonylphenyl group, 2,4-dichlorophenyl group, 2-chloro-5-(1-dodecyloxycarbonylethoxycarbonyl)phenyl group, 2-chlorophenyl group and 2-ethoxyphenyl group.

Examples of R₅₄ include a 3-{2-(2,4-di-t-amylphenoxy)butaneamido}-benzamido group, 3-{4-(2,4-di-t-amylphenoxy)butaneamido}benzamido group, 2-chloro-5-tetradecaneamidoanilino group, 5-(2,4-di-t-amylphenoxyacetamido)benzamido group, 2-chloro-5-dodecenylsuccinimidoanilino group, 2-chloro-5-{2-(3-t-butyl-4-hydroxyphenoxy)tetradecaneamido}anilino group, 2,2-dimethylpropanamido group, 2-(3-pentadecylphenoxy)butaneamido group, pyrrolidino group and N,N-dibutylamino group. Examples of R₅₅ include a 2,4,6-trichlorophenyl group, 2-chlorophenyl group, 2,5-dichlorophenyl group, 2,3-dichlorophenyl group, 2,6-dichloro-4-methoxyphenyl group, 4-{2-(2,4-di-t-amylphenoxy)butaneamido}phenyl group and 2,6-dichloro-4-methanesulfonylphenyl group. Examples of R₅₆ include a methyl group, ethyl group, isopropyl group, methoxy group, ethoxy group, methylthio group, ethylthio group, 3-phenylureido group, and 3-(2,4-di-t-amylphenoxy)propyl group. Examples of R₅₇ include a 3-(2,4-di-t-amylphenoxy)propyl group, 3-[4-{2-[4-(4-hydroxyphenylsulfonyl)phenoxy]tetradecaneamido}phenyl]propyl group, methoxy group, methylthio group, ethylthio group, methyl group, 1-methyl-2-{2-octyloxy-5-[2-octyloxy-5-(1,1,3,3-tetramethylbutyl)phenylsulfonamido]phenylsulfonamido}ethyl group, 3-{4-(4-dodecyloxyphenylsulfonamido)phenyl}propyl group, 1,1-dimethyl-2-{2-octyloxy-5-(1,1,3,3-tetramethylbutyl)phenylsulfonamido}ethyl group and dodecylthio group. Examples of R₅₈ include a 2-chlorophenyl group, pentafluorophenyl group, heptafluoropropyl group, 1-(2,4-di-t-amylphenoxy)propyl group, 3-(2,4-di-t-amylphenoxy)propyl group, 2,4-di-t-amylphenoxymethyl group and furyl group. Examples of R₅₉ include a chlorine atom, a methyl group, ethyl group, propyl group, butyl group, isopropyl group, 2-(2,4-di-t-amylphenoxy)-butaneamido group, 2-(2,4-di-t-amylphenoxy)-hexaneamido group, 2-(2,4-di-t-octylphenoxy)octaneamido group, 2-(2-chlorophenoxy) tetradecaneamido group, 2-{4-(4-hydroxyphenylsulfonyl) phenoxy}tetradecaneamido group and 2-{2-(2,4-di-t-amylphenoxyacetamido)phenoxy}butaneamido group. Examples of R₆₀ include a 4-cyanophenyl group, 2-cyanophenyl group, 4-butylsulfonylphenyl group, 4-propylsulfonylphenyl group, 4-chloro-3-cyanophenyl group, 4-ethoxycarbonylphenyl group and 3,4-dichlorophenyl group. Examples of R₆₁ include a dodecyl group, hexadecyl group, cyclohexyl group, 3-(2,4-di-t-amylphenoxy)propyl group, 4-(2,4-di-t-amylphenoxy)butyl group, 3-dodecyloxypropyl group, t-butyl group, 2-methoxy-5-dodecyloxycarbonylphenyl group and 1-naphthyl group. Examples of R₆₂ include an isobutyloxycarbonylamino group, ethoxycarbonylamino group, phenylsulfonylamino group, methanesulfonamido group, benzamido group, trifluoroacetamido group, 3-phenylureido group, butoxycarbonylamino group and acetamido group. Examples of R₆₃ include a 2,4-di-t-amylphenoxyacetamido group, 2-(2,4-di-t-amylphenoxy)butaneamido group, hexadecylsulfonamido group, N-methy-N-octadecylsulfamoyl group, N,N-dioctylsulfamoyl group, 4-t-octylbenzoyl group, dodecyloxycarbonyl group, chlorine atom, nitro group, cyano group, N-{4-(2,4-di-t-amylphenoxy)butyl}carbamoyl group, N-3-(2,4-di-t-amylphenoxy)propylsulfamoyl group, methanesulfonyl group and hexadecylsulfonyl group. Among the couplers represented by the formulas (Cp-1) to (Cp-10), cyan coupler residues represented by formulas (Cp-7) and (Cp-8) are preferred, with naphthol type cyan couplers represented by formula (Cp-8) being particularly preferred.

The timing group represented by T is a group which is cleaved from X after the cleavage of the bond between T and Cp by the coupling reaction of the coupler of formula (I) with an oxidized aromatic primary amine developing agent. The timing group is used for various purposes of controlling coupling reactivity, stabilization of the couplers, and controlling the releasing timing of the X-containing residue. Examples of the timing group include the following bonding groups.

### (1) Groups which utilize the cleavage reaction of hemiacetal

Examples of the groups include those represented by the following general formula (T-1) described in U.S. Patent 4,146,396, JP-A-60-249148 and JP-A-60-249149. In the formula (T-1), * represents the position where T is bonded to Cp in formula (I) and ** represents the position where T is bonded to X in formula (I).
wherein W represents an oxygen or sulfur atom or
R₁₁ and R₁₂ each represents a hydrogen atom or a substituent group; R₁₃ represents a substituent group; and t is 1 or 2.
When t is 2, the two
groups may be the same or different. In the case where R₁₁ and R₁₂ are each a substituent group, examples of R₁₁, R₁₂ and R₁₃ include R₁₅, R₁₅CO-, R₁₅SO₂-,
wherein R₁₅ represents an aliphatic group, an aromatic group or a heterocyclic group and R₁₆ represents a hydrogen atom, an aliphatic group, an aromatic group or a heterocyclic group. Each of R₁₁, R₁₂ and R₁₃ may be a divalent group and these bonding groups may be linked to form a ring structure. Such ring structures are included within the scope of the present invention. Examples of the groups represented by formula (T-1) include the following groups, but the present invention is not to be construed as being limited thereto.

### (2) Groups which undergo a cleavage reaction by utilizing an intramolecular nucleophilic substitution reaction

Examples of the groups include timing groups represented by the following general formula (T-2) described in U.S. Patent 4,248,292.

*-Nu-Link-E-** (T-2)

wherein Nu represents a nucleophilic group (examples of nucleophilic species being an oxygen and sulfur atoms); E represent an electrophilic group which is a group which cause the cleavage of the bond marked ** by nucleophilic attack by Nu; and Link is a linking group through which Nu and E are sterically positioned such that an intramolecular nucleophilic substitution reaction takes place. Examples of the groups represented by formula (T-2) include the following groups, but the present invention is not to be construed as being limited thereto.

### (3) Groups which undergo a cleavage reaction by utilizing an electron transfer reaction along a conjugated system

Examples of the groups include those represented by the following general formula (T-3) described in U.S. Patents 4,409,323 and 4,421,845, JP-A-57-188035, JP-A-58-98728, JP-A-58-209736, JP-A-58-209737 and JP-A-58-209738.
wherein * and **, W, R₁₁, R₁₂ and t are as defined in formula (T-1). R₁₁ and R₁₂ may be linked to form a member of a benzene ring or a heterocyclic ring. R₁₁ or R₁₂ may be combined with W to form a benzene ring or a heterocyclic ring. Z₁ and Z₂ are independently a carbon atom or a nitrogen atom; x and y are each 0 or 1. When Z₁ is carbon atom, x is 1, and when Z₁ is nitrogen atom, x is 0. The relationship between Z₂ and y is the same as that between Z₁ and x. t is 1 or 2. When t is 2, the two
groups may be the same or different.

Examples of the groups represented by the formula (T-3) include the following groups, but the present invention is not to be construed as being limited thereto.

### (4) Groups which utilize a cleavage reaction by the hydrolysis of an ester

Examples of the groups include bonding groups described in West German Patent (Laid Open) No. 2,626,315 which are groups represented by the following formulas (T-4) and (T-5).

### (5) Groups which utilize a cleavage reaction of imino-ketal

Examples of the groups include bonding groups described in U.S. Patent 4,546,073, which are groups represented by the following formula (T-6).
wherein * and ** and W are as defined and R₁₄ has the same meaning as R₁₃ in formula (T-1). Examples of the groups represented by formula (T-6) include the following groups, but the present invention is not to be construed as being limited thereto.

### (6) Groups composed of a composite structure of two or more of the above items (1) to (5).

Examples of the groups include those described in JP-A-57-56837, JP-A-60-214358, JP-A-60-218645, JP-A-60-229030, JP-A-61-156127 and JP-A-63-37346. More specifically, examples thereof include the following groups, but the present invention is not to be cosntrued as being limited thereto.

Among the above-described timing groups, the timing groups represented by formulas (T-1) to (T-3) are preferred in the present invention. As described above, ℓ is an integer of 0 or 1. However, it is preferred that ℓ is 0, that is, Cp and X are directly bonded to each other.

X in formula (I) is a divalent bonding group which is bonded to (T)_{ℓ} through N, O or S. More preferably, X is -O-, -S-,
-OSO₂-, -OSO₂NH- or a divalent group which is bonded to (T)_{ℓ} through N, such as a divalent heterocyclic group (e.g., a group derived from pyrrolidine, piperidine, morpholine, piperazine, pyrrole, pyrazole, imidazole, 1,2,4-triazole, benzotriazole, succinimide, phthalimide, oxazolidine-2,4-dione, imidazolidine-2,4-dione, or 1,2,4-triazolidine-3,5-dione) or a bonding group which is a composite group derived from these groups and an alkylene group (e.g., methylene, ethylene, trimethylene), a cycloalkylene group (e.g., 1,4-cyclohexylene), an arylene group (e.g., o-phenylene, p-phenylene), a divalent heterocyclic group (e.g., a group derived from pyridine or thiophene), -CO-, -SO₂-, -COO-, -CONH-, -SO₂NH-, -SO₂O-, -NHCO-, -NHSO₂-, -NHCONH-, -NHSO₂NH- or -NHCOO-. More preferably, X is a group represented by formula (II)

*-X₁-(L-X₂)ₘ-** (II)

In the formula (II), * represents the position where X₁ is bonded to (T)_{ℓ}; ** represents the position where X₂ is bonded to Y; X₁ represents -O- or -S-; L represents an alkylene group; X₂ represents a single bond, -O-, -S-, -CO-, -SO₂-,
-SO₂NH-, -NHSO₂-, -SO₂O-, -OSO₂-,
-NHSO₂NH-,
-OSO₂NH or -NHSO₂O-; and m is 0 or an integer of 1 to 3. The total number of carbon atom s(hereinafter referred to as the C-number) of X is preferably 0 to 12, more preferably 0 to 8.

Y in formula (I) is an arylene group or a divalent heterocyclic group. When Y is an arylene group, the arylene group may be a condensed ring, and the arylene group may have one or more substituent groups (e.g., halogen, hydroxyl, nitro, cyano, alkyl, cycloalkyl, aryl, carbonamido, sulfonamido, alkoxy, aryloxy, acyl, sulfonyl, carboxyl, sulfo, carbamoyl, sulfamoyl). The C-number is preferably 6 to 15, more preferably 6 to 10.

When Y is a divalent heterocyclic group, the heterocyclic group is a 3-membered to 8-membered (preferably 5-membered to 7-membered) monocyclic or condensed ring heterocyclic group containing at least one hetero-atom selected from the group consisting of N, O, S, P, Se and Te as a member of the heterocyclic ring (e.g., a group derived from pyridine, thiophene, furan, pyrrole, pyrazole, imidazole, thiazole, oxazole, benzothiazole, benzoxazole, benzofuran, benzothiophene, 1,3,4-thiadiazole, indole, or quinoline). The heterocyclic group may have one or more substituent groups (examples of the substituent groups include those already described above in the definition of the substituent groups for the arylene group of Y). The C-number is preferably 2 to 15, more preferably 2 to 10.

When R₁, R₂ or R₃ in formula (I) is an alkyl group, the alkyl group includes both straight-chain and branched chain alkyl groups which may have unsaturated bonds and one or more substituent groups (e.g., halogen, hydroxyl, carboxyl, sulfo, phosphono, phosphino, cyano, alkoxy, aryl, alkoxycarbonyl, amino, ammonium, acyl, carbonamido, sulfonamido, carbamoyl, sulfamoyl, or sulfonyl).

When R₁, R₂ or R₃ is a cycloalkyl group, the cycloalkyl group is a 3-membered to 8-membered cycloalkyl group which may have crosslinking groups, unsaturated bonds or substituent groups (examples of the substituent groups include those already described above in the definition of the substituent groups for the alkyl group of R₁, R₂ or R₃).

When R₁, R₂ or R₃ is an aryl group, the aryl group may be a condensed ring and may have substituent groups (examples of the substituent groups include alkyl, cycloalkyl and those already described above in the definition of the substituent groups for the alkyl group of R₁, R₂ or R₃).

When R₁, R₂ or R₃ is a heterocyclic group, the heterocyclic group is a 3-membered to 8-membered (preferably 5-membered to 7-membered) monocyclic or condensed ring heterocyclic group containing at least one hetero-atom selected from the group consisting of N, S, O, P, Se and Te as a member of the heterocyclic ring. Examples of the heterocyclic group include imidazolyl, thienyl, pyrazolyl, thiazolyl, pyridyl and quinolinyl. The heterocyclic group may have one or more substituent groups (examples of the substituent groups are the same as those for the aryl group of R₁, R₂ or R₃).

The carboxyl group includes a carboxylate group; the sulfo group includes a sulfonato group; the phosphino group includes a phosphinato group; and the phosphono group includes a phosphonato group. Those groups may include any counter ions, including Li⁺, Na⁺, K⁺ or ammonium.

Preferably, R₁ is a hydrogen atom, a carboxyl group, an alkyl group having 1 to 10 carbon atoms (e.g., methyl, t-butyl, sulfomethyl, 2-sulfoethyl, carboxymethyl, 2-carboxyethyl, 2-hydroxyethyl, benzyl, ethyl, isopropyl) or an aryl group having 6 to 12 carbon atoms (e.g., phenyl, 4-methoxyphenyl, 4-sulfophenyl) with a hydrogen atom, a methyl group or a carboxyl group being particularly preferred.

Preferably, R₂ is a cyano group, carboxyl group, a carbamoyl group having 1 to 10 carbon atoms, a sulfamoyl group having 0 to 10 carbon atoms, a sulfo group, an alkyl group having 1 to 10 carbon atoms (e.g., methyl, sulfomethyl), a sulfonyl group having 1 to 10 carbonatoms (e.g., methylsulfonyl, phenylsulfonyl), a carbonamido group having 1 to 10 carbon atoms (e.g., acetamido, benzamido) or a sulfonamido group having 1 to 10 carbon atoms (e.g., methanesulfonamido, toluenesulfonamido) with a cyano group, carbamoyl group or carboxyl group being particularly preferred.

Preferably, R₃ is a hydrogen atom, an alkyl group having 1 to 12 carbon atoms (e.g., methyl, sulfomethyl, carboxyethyl, 2-sulfoethyl, 2-carboxyethyl, ethyl, n-butyl, benzyl, 4-sulfobenzyl) or an aryl group having 6 to 15 carbon atoms (e.g., phenyl, 4-carboxyphenyl, 3-carboxyphenyl, 4-methoxyphenyl, 2,5-dicarboxyphenyl, 3,5-dicarboxyphenyl, 2-sulfophenyl, 3-sulfophenyl, 4-sulfophenyl, 2,4-disulfophenyl, 2,5-disulfophenyl). More preferably, R₃ is an alkyl group having 1 to 7 carbon atoms or an aryl group having 6 to 10 carbon atoms.

Examples of Cp, X, Y and
in formula (I) include the following groups (examples of T have been already described above), but the present invention is not construed as being limited thereto.

### Examples of Cp

### Examples of X

-O-, -S-, -OCH₂-, -OCH₂ CH₂-, -OCH₂ CH₂ O-, -OCH₂ CH₂ CH₂ O-, -O (CH₂ CH₂ O)₂-, -OCH₂ CH₂ S-, -OCH₂ CH₂ NHCO-, -OCH₂ CH₂ NHSO₂-, -OCH₂ CH₂ SO₂-, -OCH₂ CH₂ OCO-, -OCH₂ CH₂ CO-, -OCO-, -SCH₂ CONH-, -SCH₂ COO-,
-OCH₂ CH₂OSO₂-,

### Examples of Y

and

Examples of the colored couplers of the present invention include the following compounds, but the present invention is not to be construed as being limited thereto.

In the present invention, the water soluble compound (dye) comprising a 6-hydroxy-2-pyridone-5-azo group, which is released from the coupler by development processing should be dissolved out from the photographic material. The compound preferably is soluble in a developing solution of pH 9 to 12 in an amount of at least 1g/ℓ, more preferably 3g/ℓ.

The colored couplers of the present invention can be generally synthesized by the diazo coupling reaction of a 6-hydroxy-2-pyridone compound with an aromatic diazonium salt or heterocyclic diazonium salt having a coupler structure.

The former 6-hydroxy-2-pyridone compounds can be synthesized by methods described in Klinsberg, Heterocyclic Compound - Pyridine and Its Derivatives, Part 3 (Interscience 1962); J. Am. Chem. Soc., Vol. 65. page 449 (1943); J. Chem. Tech. Biotechnol., Vol. 36, page 410 (1986); Tetrahedron, Vol. 22, page 445 (1966); JP-B-61-52827 (the term "JP-B" as used herein means an "examined Japanese patent publication"); West German Patents 2,162,612, 2,349,709 and 2,902,486; and U.S. Patent 3,763,170.

The latter diazonium salts can be synthesized according to the methods described in U.S. Patents 4,004,929 and 4,138,258, JP-A-61-72244 and JP-A-61-273543. The diazo coupling reaction of the 6-hydroxy-2-pyridone compounds with the diazonium salts can be carried out in a solvent such as methanol, ethanol, methyl cellosolve, acetic acid, N,N-dimethylformamide, N,N-dimethylacetamide, tetrahydrofuran, dioxane, water or the like or a mixture thereof. In this reaction, sodium acetate, potassium acetate, sodium carbonate, potassium carbonate, sodium hydrogencarbonate, sodium hydroxide, potassium hydroxide, pyridine, triethylamine, tetramethylurea, or tetramethyl guanidine can be used as a base. The reaction temperature is generally from -78 to +60°C, preferably from -20 to +30°C.

Synthesis examples of the colored couplers of the present invention are described below.

### Synthesis Example 1

### Synthesis of Coupler (1)

### Synthesis of Compound a

125.2 g of taurine and 66 g of potassium hydroxide were added to 500 ml of methanol. The mixture was stirred with heat-refluxing. 110 g of methyl cyanoacetate was added dropwise thereto over a period of about one hour. The mixture was heated to reflux for 5 hours and then left to stand overnight. The precipitated crystal was recovered by filtration, washed with ethanol and dried to give 202.6 g of the compound a as a crystal.

### Synthesis of Compound b

11.5 g of the compound a and 3.5 g of potassium carbonate were added to 11.5 ml of water. While heating the mixture on a steam bath with stirring, 7.8 g of ethyl acetoacetate was added dropwise thereto. The mixture was stirred for 7 hours and then allowed to cool. 9.2 ml of concentrated hydrochloric acid was added thereto, whereby a crystal was precipitated. The crystal was recovered by filtration, washed with methanol and dried to give 10.4 g of the compound b as a crystal.

### Synthesis of Coupler (1)

10.1 g of compound c synthesized by the method described in U.S. Patent 4,138,258 was dissolved in 60 ml of N,N-dimethylformamide and 60 ml of methyl cellosolve. While cooling the resulting solution with ice, 4.3 ml of concentrated hydrochloric acid was added thereto and a solution of 1.84 g of sodium nitrite in 5 ml of water was added dropwise thereto to prepare a diazonium solution. 60 ml of methyl cellosolve and 20 ml of water were added to 7.8 g of the compound b and 8.2 g of sodium acetate. While stirring the resulting solution under ice cooling, the above diazonium solution was added dropwise thereto. After dropwise addition, the mixture was stirred for one hour and then at room temperature for 2 hours. The precipitated crystal was recovered by filtration, washed with water, dried and dispersed in 500 ml of methanol. The dispersion was heated to reflux for one hour and then allowed to stand to cool it. The crystal was recovered by filtration, washed with methanol and dried to give 13.6 g of the desired coupler (1) as a red crystal with a melting point of 269 to 272°C (decomposition). The structure of the compound was confirmed by ¹HNMR spectrum, mass spectrum and elemental analysis. The compound exhibited a maximum absorption wavelength in methanol at 457.7 nm and had an molecular extinction coefficient of 41300. The compound was found to have good spectral absorption characteristics as a yellow colored coupler.

### Synthesis Example 2

### Synthesis of Coupler (3)

75 ml of N,N-dimethylformamide and 75 ml of methyl cellosolve were added to 19.2 g of compound d synthesized by the method described in JP-A-62-85242 (U.S. Patent 4,837,136) to dissolve it. While stirring the resulting solution under ice cooling, 5.6 ml of concentrated hydrochloric acid was added thereto and a solution of 2.5 g of sodium nitrite in 5 ml of water was then added dropwise thereto. After dropwise addition, the mixture was stirred for one hour and then at room temperature for one hour to prepare a diazonium solution.

75 ml of methyl cellosolve and 26 ml of water were added to 10.1 g of the compound b and 10.7 g of sodium acetate. While stirring the resulting solution under ice cooling, the above diazonium solution was added dropwise thereto. After dropwise addition, the mixture was stirred for one hour and then at room temperature for 2 hours. The precipitated crystal was recovered by filtration and dispersed in 200 ml of methanol. A solution of 2.2 g of sodium hydroxide in 10 ml of water was added dropwise thereto. The mixture was stirred for 3 hours and neutralized with concentrated hydrochloric acid. The precipitated crystal was washed with water and then methanol and dried. The resulting crude crystal was purified from hot methanol in the same manner as in Synthesis Example 1 to give 14.8 g of the desired coupler (3) with a melting point of 246 to 251°C (decomposition). The structure of the compound was confirmed by ¹HNMR spectrum, mass spectrum and elemental analysis. The compound exhibited a maximum absorption wavelength in methanol at 457.6 nm and had a molecular extinction coefficient of 42700. The compound was found to have good spectral absorption characteristics as a yellow colored coupler.

### Synthesis Example 3

### Synthesis of Coupler (22)

### Synthesis of Compound e

137.1 g of anthranilic acid was added to 600 ml of acetonitrile. The mixture was heat-refluxed with stirring. 92.5 g of diketene was added dropwise thereto over a period of about one hour. The mixture was heated to reflux for one hour and cooled to room temperature. The precipitated crystal was recovered by filtration, washed with acetonitrile and dried to obtain 200.5 g of the compound e as a crystal.

### Synthesis of Compound f

199.1 g of the compound e, 89.2 g of ethyl cyanoacetate and 344 g of 28% sodium methoxide were added to 0.9 ℓ of methanol. The mixture was reacted at 120°C in an autoclave for 8 hours. After the reaction mixture was left to stand overnight, the reaction mixture was concentrated under reduced pressure. 700 ml of water was added thereto and the mixture was acidified with 230 ml of concentrated hydrochloric acid. The precipitated crystal was recovered by filtration. The resulting crude crystal was washed with a mixed solvent of ethyl acetate and acetonitrile with heating to give 152 g of the compound f.

### Synthesis of Coupler (22)

13.0 g of compound g synthesized according to the method described in U.S. Patent 4,138,258 was dissolved in 40 ml of N,N-dimethylformamide. While cooling the resulting solution with ice, 4.5 ml of concentrated hydrochloric acid was added thereto and a solution of 1.48 g of sodium nitrite in 5 ml of water was added dropwise thereto to prepare a diazonium solution. 20 ml of N,N-dimethylformamide and 15 ml of water were added to 6.0 g of compound f and 8 g of sodium acetate. While stirring the mixture under ice cooling, the above diazonium solution was added dropwise thereto. After the addition, the mixture was stirred at room temperature for 30 minutes and acidified with hydrochloric acid. The product was extracted with ethyl acetate, washed with water and concentrated under reduced pressure. The concentrate was crystallized from a mixed solvent of ethyl acetate and methanol to give 13 g of the coupler (22) as a yellow crystal.

The coupler (22) had a melting point of 154-6°C. The structure thereof was confirmed by ¹HNMR spectrum, mass spectrum and elemental analysis. The compound exhibited a maximum absorption wavelength in methanol at 458.2 nm and had a molecular extinction coefficient of 42800. The compound was found to have good spectral absorption characteristics as a yellow colored coupler.

The total amount of the coupler of formula (I) according to the present invention, which is added to the photographic material is preferably 1×10⁻⁶ to 3×10⁻³ mol/m², more preferably 1×10⁻⁵ to 1×10⁻³ mol/m². It is preferred that the coupler of the present invention is added to light sensitive silver halide emulsion layers. More preferably, the same layer contains the colored coupler of the present invention together with an uncolored coupler.

The couplers of formula (I) according to the present invention can be added in the same manner as in the addition of conventional couplers described hereinafter.

It is preferred that the colored couplers of the present invention are used in combination with cyan couplers. Examples of the cyan couplers are phenol type couplers and naphthol type couplers. Preferred examples of the cyan couplers are those described in U.S. Patents 4,052,212, 4,146,396, 4,228,233, 4,296,200, 2,369,929, 2,801,171, 2,772,162, 2,895,826, 3,772,002, 3,758,308, 4,334,011 and 4,327,173, West German Patent Application (Laid-Open) No. 3,329,729, European Patents 121,365A and 249,453A, U.S. Patents 3,446,622, 4,333,999, 4,775,616, 4,451,559, 4,427,767, 4,690,889, 4,254,212 and 4,296,199 and JP-A-61-42658.

It is more preferred that the colored couplers of the present invention are used in combination with naphthol cyan couplers. It is particularly preferred that the colored couplers of the present invention are used together with naphthol couplers represented by the following formula (C).

In formula (C), R₁ represents -CONR₄R₅, -SO₂NR₄R₅, NHCOR₄, -NHCOOR₆, -NHSO₂R₆, -NHCONR₄R₅ or -NHSO₂NR₄R₅; R₂ represents a group attached to the naphthalene ring; ℓ is 0 or an integer of 1 to 3; R₃ represents a substituent group; X represents a hydrogen atom or a group which is eliminated by the coupling reaction with an oxidized aromatic primary amine developing agent; R₄ and R₅, which may be the same or different, each represents a hydrogen atom, an alkyl group, an aryl group or a heterocyclic group; and R₆ is an alkyl group, an aryl group or a heterocyclic group. When ℓ is an integer of two or more, plural R₂ groups may be the same or different, or may be linked to form a ring. R₂ and R₃ or R₃ and X may be combined together to form a ring. They may be bonded to each other through a divalent or polyvalent group at a position of R₁, R₂, R₃ or X to form a dimer or a polymer higher than dimer.

Each substituent group in the formula (C) is now described in more detail.

R₁ is -CONR₄R₅, -SO₂NR₄R₅, -NHCOR₄, -NHCOOR₆, -NHSO₂R₆, -NHCONR₄R₅ or -NHSO₂NR₄R₅; R₄, R₅ and R₆ are each an alkyl group having 1 to 30 carbon atoms, an aryl group having 6 to 30 carbon atoms or a heterocyclic group having 2 to 30 carbon atoms and R₄ and R₅ may be a hydrogen atom.

R₂ is a group (including an atom; the same applies hereinbelow) which can be attached to the naphthalene ring. Examples of R₂ include a halogen atom (F, Cl, Br, I), a hydroxyl group, a carboxyl group, an amino group, a sulfo group, a cyano group, an alkyl group, an aryl group, a heterocyclic group, a carbonamido group, a sulfonamido group, a carbamoyl group, a sulfamoyl group, a ureido group, an acyl group, an acyloxy group, an alkoxy group, an aryloxy group, an alkylthio group, an arylthio group, an alkylsulfonyl group, an arylsulfonyl group, a sulfamoylamino group, an alkoxycarbonylamino group, a nitro group and an imido group. When ℓ=2, examples thereof include a dioxymethylene group and a trimethylene group. The number of carbon atoms of (R₂)ℓ is 0 to 30.

R₃ is a substituent group and preferably a group represented by the following formula (C-1)

R₇(Y)ₘ- (C-1)

In formula (C-1), Y is 〉NH, 〉CO or 〉SO₂; m is 0 or 1; and R₇ is a hydrogen atom, an alkyl group having 1 to 30 carbon atoms, an aryl group having 6 to 30 carbon atoms, a heterocyclic group having 2 to 30 carbon atoms, -COR₈,
-OR₁₀,
-CO₂R₁₀,
-SO₂OR₁₀ or -SO₂R₁₀. R₈, R₉ and R₁₀ have the same meaning as R₄, R₅ and R₆, respectively.

In R₁, R₄ and R₅ of
or in R₇, R₈ and R₉ of
may be combined together to form a nitrogen-containing heterocyclic ring (e.g., a pyrrolidine ring, piperidine ring, morpholine ring).

X is a hydrogen atom or a group which can be eliminated by a coupling reaction with an oxidized aromatic primary amine developing agents (a "coupling-off" group or atom). Typical examples of the coupling-off group include halogen atoms, OR₁₁, -SR₁₁,
-NHCOR₁₁,
thiocynato group and a heterocyclic group having 1 to 30 carbon atoms which is attached to the coupling active site through a nitrogen atom (e.g., a succinimido group, phthalimido group, pyrazolyl group, hydantoinyl group, or 2-benztriazolyl group). R₁₁ has the same meaning as R₆.

The above-described alkyl group may be a straight-chain, branched chain or cyclic alkyl group and may have unsaturated bonds or one or more substituent groups (examples of the substituent groups include a halogen atom, a hydroxyl group, an aryl group, a heterocyclic group, an alkoxy group, an aryloxy group, an alkylsulfonyl group, an arylsulfonyl group, an alkoxycarbonyl group, an acyloxy group and an acyl group). Typical examples of the alkyl group include methyl, isopropyl, isobutyl, t-butyl, 2-ethylhexyl, cyclohexyl, n-dodecyl, n-hexadecyl, 2-methoxyethyl, benzyl, trifluoromethyl, 3-dodecyloxypropyl and 3-(2,4-di-t-pentylphenoxy)propyl.

The aryl group may be a condensed ring (e.g., naphthyl group) and may have one or more substituent groups (examples of the substituent groups include a halogen atom, an alkyl group, an aryl group, an alkoxy group, an aryloxy group, a cyano group, an acyl group, an alkoxycarbonyl group, a carbonamido group, a sulfonamido group, a carbamoyl group, a sulfamoyl group, an alkylsulfonyl group and an arylsulfonyl group). Typical examples of the aryl group include phenyl, tolyl, pentafluorophenyl, 2-chlorophenyl, 4-hydroxyphenyl, 4-cyanophenyl, 2-tetradecyloxyphenyl, 2-chloro-5-dodecyloxyphenyl and 4-t-butylphenyl.

The heterocyclic group is a 3-membered to 8-membered monocyclic or condensed ring-form heterocyclic group containing at least one hetero-atom selected from the group consisting of O, N, S, P, Se and Te as a member of the heterocyclic ring and may have one or more substituent groups (examples of the substituent groups include a halogen atom, a carboxyl group, a hydroxyl group, a nitro group, an alkyl group, an aryl group, an alkoxy group, an aryloxy group, an alkoxycarbonyl group, an aryloxycarbonyl group, an amino group, a carbamoyl group, a sulfamoyl group, an alkylsulfonyl group and an arylsulfonyl group). Typical examples of the heterocyclic group include 2-pyridyl, 4-pyridyl, 2-furyl, 2-thienyl, benztriazole-1-yl, 5-phenyltetrazole-1-yl, 5-methylthio-1,3,4-thiadiazole-2-yl and 5-methyl-1,3,4-oxadiazole-1-yl.

Preferred substituent groups of the coupler (C) of the present invention are as follows.

Preferably, R₁ is -CONR₄R₅ or -SO₂NR₄R₅. Examples thereof include carbamoyl, N-n-butylcarbamoyl, N-n-dodecylcarbamoyl, N-(3-n-dodecyloxypropyl)carbamoyl, N-cyclohexylcarbamoyl, N-[3-(2,4-di-t-pentylphenoxy)propyl]carbamoyl, N-hexadecylcarbamoyl, N-[4-(2,4-di-t-pentylphenoxy)butyl]carbamoyl, N-(3-dodecyloxy-2-methylpropyl)carbamoyl, N-[3-(4-t-octylphenoxy)propyl]-carbamoyl, N-hexadecyl-N-methylcarbamoyl, N-(3-dodecyloxypropyl)sulfamoyl and N-[4-(2,4-di-t-pentylphenoxy)butyl]sulfamoyl. Particularly preferably, R₁ is -CONR₄R₅.

With regard to R₂, compounds where ℓ=0, that is unsubstituted compounds, are most preferred and compounds where ℓ=1 are less preferred. Preferably, R₂ is a halogen atom, an alkyl group (e.g., methyl, isopropyl, t-butyl, cyclopentyl), a carbonamido group (e.g., acetamido, pivalinamido, trifluoroacetamido, benzamido), a sulfonamido (e.g., methanesulfonamido, toluenesulfonamido) or a cyano group.

R₃ in formula (C-1) is preferably a group where m=0. More preferably, R₃ is a group of formula (C-1) where m=0 and R₇ is -COR₈ [e.g., formyl, acetyl, trifluoroacetyl, 2-ethylhexanoyl, pivaloyl, benzoyl, pentafluorobenzoyl, 4-(2,4-di-t-pentylphenoxy)butanoyl], -COOR₁₀ [e.g., methoxycarbonyl, ethoxycarbonyl, isobutoxycarbonyl, 2-ethylhexyloxycarbonyl, n-dodecyloxycarbonyl, 2-methoxyethoxycarbonyl] or -SO₂R₁₀ [ e.g., methylsulfonyl, n-butylsulfonyl, n-hexadecylsulfonyl, phenylsulfonyl, p-tolylsulfonyl, p-chlorophenylsulfonyl, trifluoromethylsulfonyl]. Particularly preferably, R₇ is -COOR₁₀.

Preferably, X is a hydrogen atom, a halogen atom, -OR₁₁ [e.g., an alkoxy group such as ethoxy, 2-hydroxyethoxy, 2-methoxyethoxy, 2-(2-hydroxyethoxy)ethoxy, 2-methylsulfonylethoxy, ethoxycarbonylmethoxy, carboxymethoxy, 3-carboxypropoxy, N-(2-methoxyethyl)carbamoylmethoxy, 1-carboxytridecyloxy, 2-methanesulfonamidoethoxy, 2-(carboxymethylthio)ethoxy or 2-(1-carboxytridecylthio)ethoxy or an aryloxy group such as 4-cyanophenoxy, 4-carboxyphenoxy, 4-methoxyphenoxy, 4-t-octylphenoxy, 4-nitrophenoxy, 4-(3-carboxypropaneamido)phenoxy or 4-acetamidophenoxy] or -SR₁₁ [e.g., an alkylthio group such as carboxymethylthio, 2-carboxymethylthio, 2-methoxyethylthio, ethoxycarbonyl methylthio, 2,3-dihydroxypropylthio or 2-(N,N-dimethylamino)ethylthio or an arylthio group such as 4-carboxyphenylthio, 4-methoxyphenylthio or 4-(3-carboxypropaneamido)phenylthio]. Among them, a hydrogen atom, a chlorine atom, an alkoxy group and an alkylthio group are particularly preferred.

The couplers of formula (C) may be in the form of a dimer or a higher polymer by combining two or more of them together through a divalent or higher valent group at a position of R₁, R₂, R₃ or X. In this case, the number of carbon atoms of each substituent group may be beyond the range described above.

When the couplers of formula (C) are in the form of a higher polymer, typical examples thereof include homopolymers or copolymers of addition polymerizable ethylenically unsaturated compounds having a cyan dye-forming coupler residue (cyan color forming monomers).

Couplers represented by the following formula (C-2) are preferred.

-(Gᵢ)_{gi}-(Hⱼ)ₕⱼ- (C-2)

In the formula (C-2), Gᵢ is a repeating monomer unit derived from a color forming monomer and a linking group represented by the following formula (C-3); Hⱼ is a repeating unit derived from a non-color forming monomer; i is a positive integer; j is 0 or a positive integer; and gi and hj are the weight fractions of Gᵢ and Hj, respectively. When i or j is 2 or greater, Gᵢ or Hᵢ is composed of two or more repeating units.

In the formula (C-3), R is a hydrogen atom, a chlorine atom or an alkyl group having 1 to 4 carbon atoms; A is -CONH-, -COO- or a substituted or unsubstituted phenylene group; B is a divalent group having carbon atoms at both terminals such as a a substituted or unsubstituted alkylene, phenylene or oxydialkylene group; L is -CONH-, -NHCONH-, -NHCOO-, -NHCO-, -OCONH-, -NH-, -COO-, -OCO-, -CO-, -O-, SO₂-, -NHSO₂- or -SO₂NH-; a, b, c are each 0 or 1; and Q is a moiety of a cyan coupler formed by removing one hydrogen atom from R₁, R₂, R₃ or X in the compound represented by formula (C).

Examples of the non-color forming ethylenic monomer represented by Hⱼ that are incapable of coupling with an oxidized aromatic primary amine developing agent include acrylic acid, α-chloroacrylic acid, α-alkylacrylic acids (e.g., methacrylic acid), amides and esters derived from these acrylic acids (e.g., acrylamide, methacrylamide, n-butylacrylamide, t-butylacrylamide, diacetone acrylamide, methyl acrylate, ethyl acrylate, n-propyl acrylate, n-butyl acrylate, t-butyl acrylate, isobutyl acrylate, 2-ethylhexyl acrylate, n-octyl acrylate, lauryl acrylate, methyl methacrylate, ethyl methacrylate, n-butyl methacrylate and β-hydroxyethyl methacrylate), vinyl esters (e.g., vinyl acetate, vinyl propionate and vinyl laurate), acrylonitrile, methacrylonitrile, aromatic vinyl compounds (e.g., styrene and derivatives thereof such as vinyltoluene, divinylbenzene, vinylacetophenone and sulfostyrene), itaconic acid, citraconic acid, crotonic acid, vinylidene chloride, vinyl alkyl ethers (e.g., vinyl ethyl ether), maleic esters, N-vinyl-2-pyrrolidone, N-vinylpyridine and 2- and 4-vinylpyridine. Acrylic esters, methacrylic esters and maleic esters are particularly preferred. These non-color forming ethylenic monomers may be used as a mixture of two or more of them. For example, a combination of methyl acrylate and butyl acrylate, a combination of butyl acrylate and styrene, a combination of butyl methacrylate and methacrylic acid or a combination of methyl acrylate and diacetone acrylamide can be used.

Ethylenically unsaturated monomers to be copolymerized with the vinyl monomers corresponding to the formula (C) can be chosen so that the forms such as solid, liquid or micelle forms of the resulting copolymers, the physical properties and/or chemical properties (e.g., solubility in water or organic solvents) thereof, the compatibility thereof with binders such as gelatin in photographic colloid compositions, flexibility, thermal stability, the coupling reactivity thereof with the oxidants of developing agents and non-diffusibility in photographic colloid are favorably affected, as is known in the field of polymer couplers. These copolymers may be any of a random copolymer and a specific sequence-copolymer (e.g., a block copolymer, an alternating copolymer).

The number-average molecular weight of the cyan polymer couplers used in the present invention is usually on the order of from several thousands to millions, but oligomer type polymers having a number-average molecular weight of 5000 or less can be used.

The cyan polymer couplers used in the present invention may be any of lipophilic polymers soluble in organic solvents (e.g., ethyl acetate, butyl acetate, ethanol, methylene chloride, cyclohexanone, dibutyl phthalate, tricresyl phosphate), hydrophilic polymers miscible with hydrophilic colloid such as an aqueous gelatin solution and polymers having a structure capable of forming a micelle in hydrophilic colloid.

It is preferred that lipophilic non-color forming ethylenic monomers (e.g., acrylic esters, methacrylic esters, maleic esters, a vinylbenzene) are mainly used as copolymerizable components to obtain the lipophilic polymer couplers soluble in organic solvents.

The lipophilic polymer couplers obtained by polymerizing the vinyl monomers giving the coupler units of formula (3-C) may be prepared by emulsifying and dispersing the solutions of the couplers in organic solvents in the form of a latex in an aqueous gelatin solution or by direct emulsion polymerization.

A method for emulsifying and dispersing the lipophilic polymer couplers in the form of latex in an aqueous gelatin solution is described in U.S. Patent 3,451,820. Emulsion polymerization can be carried out by methods described in U.S. Patents 4,080,211 and 3,370,952.

It is preferred that hydrophilic non-color forming ethylenic monomers such as N-(1,1-dimethyl-2-sulfonatoethyl)acrylamide, 3-sulfonatopropyl acrylate, sodium styrenesulfonate, potassium styrene-sulfinate, acrylamide, methacrylamide, acrylic acid, methacrylic acid, N-vinylpyrrolidone and N-vinylpyridine are used as copolymerizable components to obtain hydrophilic polymer couplers soluble in neutral or alkaline water.

The hydrophilic polymer couplers can be added to coating solutions in the form of an aqueous solution. The couplers may be dissolved in a mixed solvent of water and a water-miscible organic solvent such as a lower alcohol, tetrahydrofuran, acetone, ethyl acetate, cyclohexanone, ethyl lactate, dimethylformamide or dimethylacetamide and then added. Further, the couplers may be dissolved in an aqueous alkaline solution or an alkaline water-containing organic solvent and then added. A small amount of a surfactant may be added.

Examples of each substituent group in the formula (C) and the cyan couplers of the formula (C) include the following groups and compounds, but the present invention is not to be construed as being limited thereto.

### Examples of R₁

-CONH (CH₂)₃ O-A -CONH (CH₂)₄ O-A -CONH (CH₂)₃ OC₁₂H₂₅-(n) -CONH (CH₂)₃ OC₁₀H₂₁-(n)
-CONHC₁₆H₃₃-(n)
-CONH(CH₂ CH₂ O)₂ C₁₂H₂₅-(n) -CONHCH₂ CH₂ OC₁₂H₂₅-(n)
-CONHC₄ H₉-(n),
-CONH(CH₂)₃ OC₁₄H₂₉-(n), -CONH(CH₂)₃OC₁₁H₂₃-(n) -SO₂NH(CH₂)₃OC₁₂H₂₅-(n)
-NHCO(CH₂)₃O-A
-NHSO₂ C₁₆H₃₃-(n)
and -NHCOOC₁₂H₂₅-(n)

### Examples of R₂

-F, -Cℓ, -CN, -CH₃, -CF₃, -C₄ H₉-(t), -C₈ H₁₇-(t) -NHCOCH₃, -NHSO₂ CH₃, -NHCOOC₂ H₅
and -OC₈H₁₇-(n)

### Examples of R₃NH-

-NHCOCH₃, -NHCOCF₃,
-NHCOC₄H₉-(t) -NHCO(CH₂)₃O-A,
-NHSO₂CH₃ -NHSO₂CF₃, -NHSO₂C₄H₉-(n)
-NHCOOC₄H₉-(n), -NHCOOCH₂CH₂OCH₃
-NHCOOC₁₂H₂₅-(n) -NHCOOCH₂CH₂O-A, -NHCOCOCH₃

### Examples of X

-OC₂ H₅, -OCH₂ CH₂ OH, -OCH₂ CH₂SO₂CH₃ -O (CH₂ CH₂ O) ₂ H, -OCH₂ COOH -O (CH₂)₃ COOH, -OCH₂ COOC₂ H₅ -OCH₂ CONHCH₂ CH₂ OCH₃ -OCH₂CH₂SCH₂COOH,
-OCH₂CH₂OCH₃, -OCH₂CH₂NHSO₂CH₃
-SCH₂COOH, -SCH₂CH₂COOH
-SCH₂COOC₂H₅, -SCH₂CH₂OH
and

### Examples of Coupler (C)

### Other Couplers

In the above formulas, A represents
represents a cyclohexyl group;
represents a cyclopentyl group; and -C₈H₁₇₍ₜ₎ represents

Other examples of the cyan couplers of formula (C) which are not exemplified above and/or methods for synthesizing these compounds are described in U.S. Patent 4,690,889, JP-A-60-237448, JP-A-61-153640, JP-A-61-145557, JP-A-63-208042, JP-A-64-31159 and West German Patent 3823049A.

The photographic material of the present invention has a support having thereon at least one blue-sensitive silver halide emulsion layer, green-sensitive silver halide emulsion layer and red-sensitive silver halide emulsion layer. There is no particular limitation with regard to the number of layers of silver halide emulsion layers and non-sensitive layers and the order of the layers. A typical example is a silver halide photographic material having at least one sensitive layer composed of a plurality of silver halide emulsion layers having substantially the same color sensitivity, but different light sensitivity, the sensitive layer being a unit sensitive layer having color sensitivity to any one of blue light, green light and red light. In a multi-layer silver halide color photographic material, the unit sensitive layers are generally arranged in the order of a red-sensitive layer, a green-sensitive layer and a blue-sensitive layer from the support. However, the arrangement may be in the reverse order to that described above according to purpose. Further, the arrangement may be such that a different light-sensitive layer is inserted into the same color sensitive layers.

Non-sensitive layers such as various interlayers may be provided between silver halide sensitive layers, or on the uppermost layer or lowermost layer thereof.

The interlayers may contain couplers, or DIR compounds described in JP-A-61-43748, JP-A-59-113438, JP-A-59-113440, JP-A-61-20037 and JP-A-61-20038. The interlayers may also contain color mixing inhibitors as used conventionally.

A plurality of silver halide emulsion layers which constitute each unit sensitive layer preferably include a two-layer structure consisting of a high-sensitivity emulsion layer and a low-sensitivity emulsion layer as described in West German Patent 1,121,470 and U.K. Patent 923,045. It is preferred that the layers are disposed such that light sensitivity is lower toward the support. A non-sensitive layer may be provided between silver halide emulsion layers. The low-sensitivity emulsion layer may be provided on the farther side from the support and the high-sensitivity emulsion layer may be provided on the side nearer to the support as described in JP-A-57-112751, JP-A-62-200350, JP-A-62-206541 and JP-A-62-206543.

In specific embodiments, the layer may be arranged in order of low-sensitivity blue-sensitive layer (BL)/high-sensitivity blue-sensitive layer (BH)/high-sensitivity green-sensitive layer (GH)/low-sensitivity green-sensitive layer (GL)/high-sensitivity red-sensitive layer (RH)/low-sensitivity red-sensitive layer (RL) from the outermost layer, or in order of BH/BL/GL/GH/RH/RL, or in order of BH/BL/GH/GL/RL/RH.

The arrangement may be made in order of blue-sensitive layer/GH/RH/GL/RL from the outermost layer as described in JP-B-55-34932. Further, the arrangement may be made in order of blue-sensitive layer/GL/RL/GH/RH from the outermost layer as described in JP-A-56-25738 and JP-A-62-63936.

In another embodiment, the layer structure contains three layers having different light sensitivity in such an arrangement that the upper layer is a silver halide emulsion layer having the highest light sensitivity, the medium layer is a silver halide emulsion layer having a light sensitivity lower than that of the upper layer and the lower layer is a silver halide emulsion layer having a light sensitivity lower than that of the medium layer so that light sensitivity becomes lower toward the support in order as described in JP-B-49-15495. Even when the layer structure is composed of three layers having different light sensitivity, the arrangement may be made in order of medium-sensitive emulsion layer/high-sensitivity emulsion layer/low-sensitivity emulsion layer from the outermost layer.

In still another embodiment, the arrangement may be made in order of high-sensitivity emulsion layer/low sensitivity emulsion layer/medium-sensitivity emulsion layer or in order of low sensitivity emulsion layer/medium-sensitivity emulsion layer/high-sensitivity emulsion layer.

When the layer structure is composed of four or more layers, the above-described various arrangements can be made.

Various layer structures and arrangements can be chosen according to the purpose of each photographic material.

The preferred silver halide contained in the photographic emulsions of the photographic materials of the present invention is silver iodobromide, silver iodochloride or silver iodochlorobromide, each having a silver iodide content of not higher than about 30 mol%. Particularly preferred is silver iodobromide or silver iodochlorobromide, each having a silver iodide content of about 2 mol% to about 25 mol%.

Silver halide grains in the photographic emulsions may have a regular crystal form such as cube, octahedron or tetradecahedron, an irregular crystal form such as a sphere or tabular form, a crystal having a defect such as a twinning plane or a composite form thereof.

The size of silver halide grains may be in the range of from fine grains having a grain size of not larger than about 0.2 µm to large-size grains having a grain size of about 10 µm in terms of the diameter of projected area. Any of a polydisperse emulsion and monodisperse emulsion may be used.

The silver halide photographic emulsions of the present invention can be prepared according to the methods described in Research Disclosure (RD) No. 17643 (December 1978) pp 22-23 I. Emulsion Preparation and Types; ibid. No. 18716 (November 1979), p. 648; ibid. No. 307105 (November 1989), pp 863-865; P. Glafkides, Chimie et Phisique Photographique (Paul Montel 1967), G.F. Duffin, Photographic Emulsion Chemistry (Focal Press 1966) and V.L. Zelikman et al, Making and Coating Photographic Emulsion (Focal Press 1964).

Monodisperse emulsions described in U.S. Patents 3,574,628 and 3,655,394 and U.K. Patent 1,413,748 are also preferred.

Tabular grains having an aspect ratio of not lower than about 3 can be used in the present invention. The tabular grains can be easily prepared by the methods described in Gutoff, Photographic Science and Engineering, Vol. 14, pp 248-257 (1970), U.S. Patents 4,434,226, 4,414,310, 4,433,048 and 4,439,520 and U.K. Patent 2,112,157.

Grains having a uniform crystal structure or a crystal structure different in halogen composition between the interior thereof and the surface thereof can be used. Grains having a laminar crystal structure may be used. Silver halide having a different composition may be joined to the grains by epitaxial growth. A compound such as silver rhodanide or lead oxide other than silver halide may be joined to the grains. A mixture of grains having various crystal forms may be used.

There can be used any of a surface latent image type emulsion wherein a latent image is predominantly formed on the surface of grain, an internal latent image type emulsion wherein a latent image is predominantly formed in the interior of grain, and a type wherein a latent image is formed on the surface of grain as well as in the interior thereof. However, the emulsions must be negative type. The internal latent image type emulsion may be a core/shell type internal latent image type emulsion described in JP-A-63-264740. A method for preparing the core/shell type internal latent image type emulsion is described in JP-A-59-133542. The thickness of the shell of the emulsion varies depending on processing conditions, but is preferably 3 to 40 nm, particularly preferably 5 to 20 nm.

Silver halide emulsions are usually subjected to physical ripening, chemical ripening and spectral sensitization and then used. Additives used for these stages are described in Research Disclosure No. 17643, ibid. No. 18716 and ibid. No. 30716 and listed in a Table below.

In the photographic materials of the present invention, two or more emulsions differing in at least one of grain size, grain size distribution, halogen composition, grain form and sensitivity of the sensitive silver halide emulsion, can be mixed in the same layer.

Silver halide grains wherein the surfaces of grains are fogged as described in U.S. Patent 4,082,553, silver halide grains wherein the interiors of grains are fogged as described in U.S. Patent 4,626,498 and JP-A-59-214852 and colloidal silver can be preferably used in light-sensitive silver halide emulsion layers and/or substantially non-light-sensitive hydrophilic colloid layers. The term "silver halide grains wherein the interiors or surfaces of grains are fogged" as used herein refers to silver halide grains which can be developed uniformly (non-imagewise) irrespective of the unexposed area or exposed area of the photographic material. Methods for preparing silver halide grains wherein the interiors or surfaces of the grains are fogged are described in U.S. Patent 4,626,498 and JP-A-214852.

The silver halide which forms the internal nucleus of the core/shell type silver halide grains wherein the interiors of the grains are fogged, may be grains having the same halogen composition or different halogen compositions. Any of silver chloride, silver chlorobromide, silver iodobromide and silver chloroiodobromide can be used as silver halide wherein the interiors or surfaces of the grains are fogged. Though there is no particular limitation with regard to the grain size of these fogged silver halide grains, mean grain size is preferably 0.01 to 0.75 µm, particularly preferably 0.05 to 0.6 µm. There is no particular limitation with regard to the shape of grains. Grains may have a regular crystal form, and the emulsion may be polydisperse emulsion, but a monodisperse emulsion is preferred in which at least 95% (in terms of weight or the number of grains) of silver halide grains is composed of grains having a grain size within the mean grain size ±40%.

It is preferred that non-light-sensitive finely divided silver halide grains are used in the present invention. The term "non-sensitive finely divided silver halide grains" as used herein refers to finely divided silver halide grains which are not light-sensitive during imagewise exposure for obtaining a dye image and are substantially not developed in the processing stage. Grains which are previously not fogged are preferable.

Finely divided silver halide grains have a silver bromide content of 0 to 100 mol% and may optionally contain silver chloride and/or silver iodide. Grains containing 0.5 to 10 mol% of silver iodide are preferred.

Finely divided silver halide grains have a mean grain size (the mean value of diameters of the circles having areas corresponding to projected areas) of preferably 0.01 to 0.5 µm, more preferably 0.02 to 0.2 µm.

Finely divided silver halide grains can be prepared in the same manner as in the preparation of usual light-sensitive silver halides. In the preparation of finely divided silver halide grains, it is not necessary that the surfaces of silver halide grains be optically sensitized or spectrally-sensitized. However, it is preferred that a conventional stabilizer such as triazole, azaindene, benzthiazolium, a mercapto compound or a zinc compound be added before the finely divided silver halide grains are added to coating solutions. Colloidal silver is preferably incorporated in layers containing the finely divided silver halide grains.

The coating weights of coating solutions to be coated on the photographic materials of the present invention are preferably not more than 6.0 g/m², more preferably not more than 4.5 g/m² in terms of silver.

Conventional photographic additives which can be used in the present invention are described in the three Research Disclosures are listed in the following Table.

It is preferred that compounds capable of reacting with formaldehyde to fix it as described in U.S. Patents 4,411,987 and 4,435,503 are added to photographic materials to prevent photographic performance from being deteriorated by formaldehyde gas.

It is preferred that mercapto compounds described in U.S. Patents 4,740,454 and 4,788,132, JP-A-62-18539 and JP-A-1-283551 are incorporated in the photographic materials of the present invention.

Preferably, the photographic materials of the present invention contain fogging agents, development accelerators and solvents for silver halide or compounds releasing their precursors as described in JP-A-1-106052, irrespective of the amount of developed silver formed by development.

It is also preferred that dyes dispersed by the methods described in WO88/04794 and Published PCT Application No. 502912/1989 (in Japan) or dyes described in EP317,308A, U.S. Patent 4,420,555 and JP-A-1-259358 are incorporated in the photographic materials of the present invention.

Various color couplers can be used in the present invention. Examples thereof are described in patent specifications cited in the above-described Research Disclosure No. 17643, VII-C to G and ibid. No. 307105, VII-C to G.

Preferred examples of yellow couplers include those described in U.S. Patents 3,933,501, 4,022,620, 4,326,024, 4,401,752 and 4,248,961, JP-B-58-10739, U.K. Patents 1,425,020 and 1,476,760, U.S. Patents 3,973,968, 4,314,023 and 4,511,649 and European Patent 249,473A.

5-Pyrazolone compounds and pyrazoloazole compounds are preferred as magenta couplers. Particularly preferred are magenta couplers described in U.S. Patents 4,310,619 and 4,351,897, European Patent 73,636, U.S. Patents 3,061,432 and 3,725,067, Research Disclosure No. 24220 (June 1984), JP-A-60-33552, Research Disclosure No. 24230 (June 1984), JP-A-60-43659, JP-A-61-72238, JP-A-60-35730, JP-A-55-118034, JP-A-60-185951, U.S. Patents 4,500,630, 4,540,654 and 4,556,630 and WO88/04795.

As cyan couplers other than those represented by formula (C), preferred cyan couplers include those described in U.S. Patents 4,052,212, 4,146,396, 4,228,233, 4,296,200, 2,369,929, 2,801,171, 2,772,162, 2,895,826, 3,772,002, 3,758,308, 4,334,011 and 4,327,173, West German Patent Application (Laid-Open) No. 3,329,729, European Patents 121,365A and 249,453A, U.S. Patents 3,446,622, 4,333,999, 4,775,616, 4,451,559, 4,427,767, 4,254,212 and 4,296,199 and JP-A-61-42658.

Typical examples of dye-forming polymerized couplers are described in U.S. Patents 3,451,820, 4,080,211, 4,367,282, 4,409,320 and 4,576,910, U.K. Patent 2,102,137 and European Patent 341,188A.

As couplers forming developed dyes with controlled diffusion, there are preferred those described in U.S. Patent 4,366,237,U.K. Patent 2,125,570, European Patent 96,570 and West German Patent Application (Laid-Open) No. 3,234,533.

In addition to the couplers capable of releasing a compound residue having a water-soluble 6-hydroxy-2-pyridone-5-azo group according to the present invention, there are preferred compounds described in Research Disclosure No. 17643, item VII-G, ibid. No. 307105, item VII-G, U.S. Patent 4,163,670, JP-B-57-39413, U.S. Patents 4,004,929 and 4,138,258 and U.K. Patent 1,146,368, as colored couplers for correcting the unnecessary absorption of developed dyes. It is also preferred to use couplers for correcting the unnecessary absorption of developed dyes by fluorescent dyes released during coupling as described in U.S. Patent 4,774,181 or couplers having, as an elimination group, a dye precursor group capable of reacting with developing agents to form a dye as described in U.S. Patent 4,777,120.

Compounds which release a photographically useful residue with coupling can be preferably used in the present invention. Preferred DIR couplers which release restrainers are described in patent specifications cited in the above-described RD No. 17643, item VII-F, ibid. No. 307105, item VII-F, JP-A-57-151944, JP-A-57-154234, JP-A-60-184248, JP-A-63-37346, JP-A-63-37350, U.S. Patents 4,248,962 and 4,782,012.

As couplers which release imagewise nucleating agents or development accelerators during development, there are preferred those described in U.K. Patents 2,097,140 and 2,131,188, JP-A-59-157638 and JP-A-59-170840. Compounds which release fogging agent, development accelerator and solvents for silver halide by a redox reaction with oxidized developing agents as described in JP-A-60-107029, JP-A-60-252340, JP-A-1-44940 and JP-A-1-45687 are also preferred.

Other examples of compounds which can be used in the present invention include competitive couplers described in U.S. Patent 4,130,427, polyequivalent type couplers described in U.S. Patents 4,283,472, 4,338,393 and 4,310,618, couplers releasing DIR redox compounds, couplers releasing DIR couplers, redox compounds releasing DIR couplers and redox compounds releasing DIR redox compounds described in JP-A-60-185950 and JP-A-62-24252, couplers which release dyes capable of again forming color after elimination described in European Patents 173,302A and 313,308A, couplers releasing bleaching accelerators described in RD No. 11449, RD No. 24241 and JP-A-61-201247, couplers releasing ligands described in U.S. Patent 4,555,477, couplers releasing leuco dyes described in JP-A-63-75747, and couplers releasing fluorescent dyes described in U.S. Patent 4,774,181.

Couplers used in the present invention can be introduced into photographic materials by various known dispersion methods.

Examples of high-boiling solvents used for the oil-in-water dispersion method are described in U.S. Patent 2,322,027.

Examples of the high-boiling organic solvents which have a boiling point of not lower than 175°C at normal pressure used in the oil-in-water dispersion method include phthalic esters (e.g., dibutyl phthalate, dicyclohexyl phthalate, di-2-ethylhexyl phthalate, decyl phthalate, bis(2,4-di-t-amylphenyl) phthalate, bis(2,4-di-t-amylphenyl) isophthalate, bis(1,1-diethylpropyl) phthalate), phosphoric or phosphonic esters (e.g., triphenyl phosphate, tricresyl phosphate, 2-ethylhexyl diphenyl phosphate, tricyclohexyl phosphate, tri-2-ethylhexyl phosphate, tridodecyl phosphate, tributoxyethyl phosphate, trichloropropyl phosphate, di-2-ethylhexyl phenyl phosphate,), benzoic esters (e.g., 2-ethylhexyl benzoate, dodecyl benzoate, 2-ethylhexyl p-hydroxybenzoate), amides (e.g., N,N-diethyldodecaneamide, N,N-diethyllaurylamide, N-tetradecylpyrrolidone), alcohols or phenols (e.g., isostearyl alcohol, 2,4 di-tert-amylphenol), aliphatic carboxylic acid esters (e.g., bis(2-ethylhexyl) sebacate, dioctyl azelate, glycerol tributyrate, isostearyl lactate, trioctyl citrate), aniline derivatives (e.g., N,N-dibutyl-2-butoxy-5-t-octylaniline) and hydrocarbons (e.g., paraffin, dodecylbenzene, diisopropylnaphthalene). Organic solvents having a boiling point of not lower than about 30°C, preferably not lower than about 50°C, but not higher than about 160°C can be used as co-solvents. Examples of the co-solvents include ethyl acetate, butyl acetate, ethyl propionate, methyl ethyl ketone, cyclohexanone, 2-ethoxyethyl acetate and dimethylformamide.

Examples of steps for latex dispersion methods, effects thereof and the impregnating latex are described in U.S. Patent 4,199,363, West German Patent Application (OLS) Nos. 2,541,274 and 2,541,230.

It is preferred that antiseptic and antifungal agents such as 1,2-benzoisothiazoline-3-one, n-butyl p-hydroxybenzoate, phenol, 4-chloro-3,5-dimethylphenol, 2-phenoxyethanol and 2-(4-thiazolyl)benzimidazole described in JP-A-63-257747, JP-A-62-272248 and JP-A-1-80941 and phenethyl alcohol are added to the color photographic materials of the present invention.

The present invention can be applied to various color photographic materials. Typical examples of the color photographic materials according to the present invention include general-purpose and movie color negative films, reversal color films for slide or TV, color paper, color positive films and reversal color paper.

Examples of supports which can be used in the present invention include those described in the above-described RD No. 17643 (page 28), RD No. 18716 (right column of page 647 to left column of page 648) and RD No. 307105 (page 879).

In the photographic material of the present invention, the total of the layer thicknesses of the entire hydrophilic colloid layers on the emulsion layer side thereof is preferably not more than 28 µm, more preferably not more than 23 µm, still more preferably not more than 18 µm, particularly preferably not more than 16 µm. The layer-swelling rate T_{1/2} is preferably not longer than 30 seconds, more preferably not longer than 20 seconds. The layer thickness refers to a layer thickness obtained by measuring the thickness of a layer at 25°C and 55% RH under air conditioning (2 days). The layer-swelling rate T_{1/2} can be measured by known method in the field of photography, for example, by using a swellometer described in A. Green et al., Photogr. Sci. Eng., Vol. 19, No. 2, pp. 124-129. T_{1/2} is defined as the time taken until layer thickness reaches 1/2 of saturated layer thickness when processing is conducted with a color developing solution at 30°C for 3 min 15 sec and 90% of the attainable maximum swollen layer thickness is referred to as saturated layer thickness.

The layer-swelling rate T_{1/2} can be controlled by adding a hardening agent to gelatin as a binder or by changing conditions with time after coating. A swelling ratio of 150 to 400% is preferred. The swelling ratio can be calculated from the maximum swollen layer thickness under the above conditions by using the formula (maximum swollen layer thickness - layer thickness)/layer thickness.

It is preferred that the photographic material of the present invention be provided with hydrophilic layer (referred to as a backing layers having a total dry thickness of 2 to 20 µm on the opposite side to the emulsion layer side. It is preferred that the backing layer contain a light absorber, filter dye, ultraviolet light absorber, antistatic agent, hardening agent, binder, plasticizer, lubricant, coating aid, and surfactant. The swelling ratio of the backing layer is preferably 150 to 500%

The color photographic materials of the present invention can be developed according to conventional methods described in RD No. 17643 (pp 28-29), RD No. 18716 (left column to right column of page 651) and RD No. 307105 (pp 880-881).

Color developing solutions which can be used in the processing of the photographic materials of the present invention are preferably aqueous alkaline solutions mainly composed of aromatic primary amine color developing agents. Aminophenol compounds are useful as the color developing agents and p-phenylenediamine compounds are preferred as the color developing agents. Typical examples thereof include 3-methyl-4-amino-N,N-diethylaniline, 3-methyl-4-amino-N-ethyl-N-β-hydroxyethylaniline, 3-methyl-4-amino-N-ethyl-N-β-methanesulfonamidoethylaniline, 3-methyl-4-amino-N-ethyl-N-β-methoxyethylaniline and salts thereof such as sulfate, hydrochloride and p-toluenesulfonate. Among them, 3-methyl-4-amino-N-ethyl-N-β-hydroxyethylaniline sulfate is particularly preferred. These compounds may be used either alone or in combination of two or more of them according to purpose.

Generally, the color developing solutions contain pH buffering agents such as alkali metal carbonates, borates and phosphates, developed restrainers such as chlorides, bromides, iodides, benzimidazoles, benzothiazoles and mercapto compounds and anti-fogging agents. If desired, the color developing solutions may optionally contain preservatives such as hydroxylamine, diethylhydroxylamine, sulfites, hydrazine such as N,N-biscarboxymethylhydrazine, phenylsemicarbazides, triethanolamine, catecholsulfonic acids; organic solvents such as ethylene glycol and diethylene glycol; development accelerators such as benzyl alcohol, polyethylene glycol, quaternary ammonium salts and amines; color forming couplers, competitive couplers; auxiliary developing agents such as 1-phenyl-3-pyrazolidone; tackifiers; and chelating agents such as aminopolycarboxylic acids, aminopolyphosphonic acids, alkylphosphonic acids and phosphonocarboxylic acids, for example, ethylenediaminetetraacetic acid, nitrilotriacetic acid, diethylenetriaminepentaacetic acid, cyclohexanediaminetetraacetic acid, hydroxyethyliminodiacetic acid, 1-hydroxyethylidene-1,1-diphosphonic acid, nitrilo-N,N,N-trimethylenephosphonic acid, ethylenediamine-N,N,N′,N′-tetramethylenephosphonic acid and ethylenediamine-di(o-hydroxyphenylacetic acid) and salts thereof.

Generally, when reversal processing is to be conducted, black-and-white development is first carried out and color development is then carried out. Black-and-white developing solutions may contain conventional developing agents such as dihydroxybenzenes (e.g., hydroquinone), 3-pyrazolidones (e.g., 1-phenyl-3-pyrazolidone) and aminophenols (e.g., N-methyl-p-aminophenol). These developing agents may be used either alone or in combination of two or more of them.

The pH of the color developing solutions and the black-and-white developing solutions is generally in the range of 9 to 12. The replenishment rate of these developing solutions varies depending on the types of the color photographic materials, but is usually not more than 3 ℓ per m² of the photographic material. The replenishment rate can be reduced to 500 ml or less when the concentration of bromide ion in the replenisher is reduced. When the replenishment is to be reduced, it is desirable that the contact area of the processing solution with air be reduced to prevent the solution from being evaporated or oxidized by air. The contact area of the photographic processing solution with air in the processing tank is represented by opening ratio defined below.$\text{Opening ratio =} \frac{\text{Contact area (cm²) of processing solution with air}}{\text{Capacity (cm³) of processing solution}}$

The opening ratio is preferably not higher than 0.1, more preferably 0.001 to 0.05. Methods for reducing the opening ratio include a method wherein a cover such as a floating lid is provided on the surface of the photographic processing solution in the processing tank; a method wherein a movable lid is used as described in JP-A-1-82033; and a slit development method described in JP-A-63-216050. It is preferred the opening ratio be reduced not only for color development and black and white development stages, but also all of the subsequent stages such as bleaching, bleaching-fixing, fixing, rinsing and stabilization stages. The replenishment rate can be reduced by inhibiting the accumulation of bromide ion in the developing solution.

Color development is usually 2 to 5 minutes. However, when a higher temperature and a higher pH are used and the color developing agents are used at a higher concentration, processing time can be shortened.

After color development, the photographic emulsion layer is generally bleached. Bleaching may be carried out simultaneously with fixing (bleaching-fixing treatment) or separately carried out. After bleaching, a bleaching-fixing treatment may be conducted to expedite processing. Processing may be conducted with a bleaching-fixing bath composed of two consecutive baths. Fixing may be conducted before the bleaching-fixing treatment. After the bleaching-fixing treatment, bleaching may be conducted according to purpose. Examples of bleaching agents include compounds of polyvalent metals such as iron(III), peracids, quinones and nitro compounds. Typical examples of the bleaching agents include organic complex salts of iron(III) such as complex salts of aminopolycarboxylic acids (e.g., ethylenediaminetetraacetic acid, diethylenetriaminepentaacetic acid, cyclohexanediaminetetraacetic acid, methyliminodiacetic acid, 1,3-diaminopropanetetraacetic acid, glycol ether diaminetetraacetic acid), citric acid, tartaric acid, and malic acid. Among them, iron(III) complex salts of aminopolycarboxylic acids such as (ethylenediaminetetraacetonato)-iron(III) complex and (1,3-diaminopropanetetraacetonato)iron(III) complex are preferred for rapid processing and prevention of environmental pollution. Further, iron(III) complex salts of aminopolycarboxylic acids are useful for bleaching solutions and bleaching-fixing solutions. The pH of the bleaching solutions containing the iron(III) complex salts of aminopolycarboxylic acids and the bleaching-fixing solutions containing the iron(III) complex salts is generally in the range of 4.0 to 8. A lower pH may be used to expedite processing.

If desired, the bleaching solution, the bleaching-fixing solution and the pre-bath thereof may contain bleaching accelerators. Examples of the bleaching accelerators include compounds having a mercapto group or disulfide group described in U.S. Patent 3,893,858, West German Patents 1,290,812 and 2,059,988, JP-A-53-32736, JP-A-53-57831, JP-A-53-37418, JP-A-53-72623, JP-A-53-95630, JP-A-53-95631, JP-A-53-104232, JP-A-53-124424, JP-A-53-141623, JP-A-53-28426 and Research Disclosure No. 17129 (July 1978); thiazolidine derivatives described in JP-A-50-140219; thiourea derivatives described in JP-B-45-8506, JP-A-52-20832, JP-A-53-32735 and U.S. Patent 3,706,561; iodides described in West German Patent 1,127,715 and JP-A-58-16235; polyoxyethylene compounds described in West German Patents 996,410 and 2,748,430; polyamine compounds described in JP-B-45-8836; compounds described in JP-A-49-40943, JP-A-49-59644, JP-A-53-94927, JP-A-54-35727, JP-A-55-26506 and JP-A-58-163940; and bromide ions. Among them, the compounds having a mercapto group or disulfide group are preferred for their high accelerating effect. Particularly, the compounds described in U.S. Patent 3,893,858, West German Patent 1,290,812 and JP-A-53-95630 are preferred. Further, the compounds described in U.S. Patent 4,552,834 are preferred. These bleaching accelerators may be incorporated in the photographic materials. These bleaching accelerators are particularly effective in conducting bleaching-fixing of the color photographic materials for photographing.

It is preferred that in addition to the above-described compounds, the bleaching solution and the bleaching-fixing solution contain organic acids to prevent stain from being caused by bleaching. Particularly preferred organic acids are compounds having an acid dissociation constant (pKa) of 2 to 5. Examples of the organic acids include acetic acid and propionic acid.

Examples of fixing agents used in the fixing solution and the bleaching-fixing solution include thiosulfates, thiocyanates, thioether compounds, thioureas and a large amount of an iodide. The thiosulfates are widely used as the fixing agents. Particularly, ammonium thiosulfate is most widely used. A combination of a thiosulfate with a thiocyanate, a thioether compound or a thiourea is also preferred. Sulfites, bisulfites, carbonyl bisulfite adducts and sulfinic acid compounds described in European Patent 294769A are preferred as preservatives for the fixing solution and the bleaching-fixing solution. It is also preferred that aminopolycarboxylic acids or organic phosphonic acids are added to the fixing solution or the bleaching-fixing solution to stabilize the solution.

It is preferred that compounds having a pKa of 6.0 to 9.0, preferably imidazoles such as imidazole, 1-methylimidazole, 1-ethylimidazole and 2-methylimidazole, in an amount of 0.1 to 10 mol/ℓ are added to the fixing solution or the bleaching-fixing solution to adjust the pH.

Shorter desilvering time (in total) is preferred, so long desilvering failure is not caused. Desilvering time is preferably 1 to 3 min, more preferably 1 to 2 min. Processing temperature is 25 to 50°C, preferably 35 to 45°C. When desilvering is carried out at a temperature within the preferred range, the desilvering rate is increased and stain is effectively prevented from being formed after processing.

It is preferred that agitation in the desilvering stage be intensified as much as possible. Methods for intensifying agitation include a method wherein a jet of the processing solution collides with the surfaces of the emulsions of photographic materials as described in JP-A-62-183460; a method wherein stirring is improved by a rotating means as described in JP-A-62-183461; a method wherein a wiper blade provided in the solution is brought into contact with the surfaces of the emulsions, the photographic material is transferred to thereby form a turbulent flow, whereby a stirring effect is improved; and a method wherein the whole amount of the processing solution circulated is increased. Such means for improving agitation are effectively applicable to any of the bleaching solution, the bleaching-fixing solution and the fixing solution. It is believed that an improvement agitation accelerates the feed of the bleaching solution and the fixing solution into the emulsion layers and as a result, the desilvering rate is enhanced. The above-described means for improving agitation is more effective when the bleaching accelerators are used. The accelerating effect can be greatly increased and the problem of inhibiting fixation caused by the bleaching accelerators can be solved.

It is preferred that automatic processors for use in the processing of the photographic materials of the present invention be provided with photographic material conveying means described in JP-A-60-191257, JP-A-60-191258 and JP-A-60-191259. As stated in JP-A-60-191257 the conveying means can greatly reduce the amount of the processing solution brought over from the previous bath to the subsequent bath so that preservation of the performance of the processing solution is very high. This is particularly effective in shortening the processing time in each stage or reducing the replenishment rate of the processing solution.

Usually, the silver halide color photographic materials of the present invention are subjected to washing and/or stabilization after desilvering. The amount of rinsing water in the washing stage varies widely depending on the characteristics (e.g., depending on materials used such as couplers) of the photographic materials, their use, the temperature of rinsing water, the number of rinsing tanks (the number of stages), replenishing system (countercurrent, direct flow) and other conditions. The relationship between the amount of water and the number of rinsing tanks in the multi-stage countercurrent system can be determined by the method described in Journal of the Society of Motion Picture and Television Engineers, Vol. 64, p. 248-253 (May 1955).

According to the multi-stage countercurrent system described in the above article, the amount of rinsing water can be greatly reduced. However, the residence time of water in the tanks is prolonged and as a result, bacteria are grown and the resulting suspended matter is deposited on the photographic material. A method for reducing calcium ion and magnesium ion concentrations described in JP-A-62-288838 can be effectively used for the color photographic materials of the present invention to solve this problem. Further, isothiazolone compounds, thiabendazole compounds, chlorine-containing germicides such as sodium chlorinated isocyanurate and benztriazole described in JP-A-57-8542 and germicides described in Chemistry of Germicidal Antifungal Agent, (1986) written by Hiroshi Horiguchi (Sankyo Shuppan), Sterilization, Disinfection, Antifungal Technique, edited by Sanitary Technique Society and Antibacterial and Antifungal Cyclopedie, (1986) edited by Nippon Antibacterial Antifungal Society, can be used.

The pH of rinsing water in the treatment of the photographic materials of the present invention is in the range of 4 to 9, preferably 5 to 8. The temperature of rinsing water and washing time vary depending on the characteristics of the photographic materials and use, but the temperature and time of washing are generally 15 to 45°C for 20 seconds to 10 minutes, preferably 25 to 40°C for 30 seconds to 5 minutes. The photographic materials of the present invention may be processed directly with stabilizing solutions in place of rinsing water. Such stabilizing treatment can be carried out by conventional methods described in JP-A-57-8543, JP-A-58-14834 and JP-A-60-220345.

A stabilizing treatment subsequent to rinsing may be conducted. The stabilizing treatment may be used as the final bath for the color photographic materials for photographing. An example thereof include a stabilizing bath containing a dye stabilizer and a surfactant. Examples of the dye stabilizer include aldehydes such as formalin and glutaraldehyde, N-methylol compounds, hexamethylenetetramine and aldehyde-sulfite adducts.

The stabilizing bath may contain various chelating agents and antifungal agents.

Overflow solution from the replenishment of rinsing water and/or stabilizing can be reused in other stages such as desilvering stage.

When the processing solutions are concentrated by evaporation in processing with automatic processors, it is preferred that water is added thereto to make up the amount of water evaporated.

The color developing agents may be incorporated in the silver halide color photographic materials of the present invention for the purpose of simplifying and expediting processing. It is preferred that precursors for the color developing agents are used for the incorporation thereof in the photographic materials. Examples of the precursors include indoaniline compounds described in U.S. Patent 3,342,597; Schiff base compounds described in U.S. Patent 3,342,599 Research Disclosure No. 14850 and ibid., No. 15159; aldol compounds described in Research Disclosure No. 13924; metal complex salts described in U.S. Patent 3,719,492; and urethane compounds described in JP-A-53-135628.

If desired, 1-phenyl-3-pyrazolidones may be incorporated in the silver halide color photographic materials of the present invention for the purpose of accelerating color development. Typical examples of the compounds include those described in JP-A-56-64339, JP-A-57-144547 and JP-A-58-115438.

In the present invention, various processing solutions are used at a temperature of 10 to 50°C. Generally, a temperature of 33 to 38°C is used. However, a higher temperature can be used to accelerate processing and to shorten processing time, while a lower temperature is used to improve image quality and to improve the stability of the processing solutions.

The silver halide photographic materials of the present invention include heat developable photosensitive materials described in U.S. Patent 4,500,626, JP-A-60-133449, JP-A-59-218443, JP-A-61-238056 and European Patent 210,660A2.

The present invention is now illustrated in greater detail with reference to the following examples which, however, are not to be construed as limiting the invention in any way. Unless otherwise indicated, all parts, percents and ratios are by weight.

### EXAMPLE 1

The surface of a triacetyl cellulose film support having an undercoat layer applied thereto was coated with each of the following layers having the following compositions to prepare a photographic material 101.

### (1) Emulsion Layer

### (2) Protective Layer

### Sample 102

A sample 102 was prepared in the same way as in the preparation of the sample 101 except that comparative colored coupler R-1 in an amount of 0.08 g/m² was added to the emulsion layer.

### Samples 103 to 107

Each of samples 103 to 107 was prepared in the same way as in the preparation of the sample 102 except that an equimolar amount of each of couplers indicated in Table 1 was used in place of the coupler R-1.

### Sample 108

A sample 108 was prepared in the same way as in the preparation of the sample 104 except that tricresyl phosphate was omitted from the emulsion layer.

### Samples 109 to 111

Each of samples 109 to 111 was prepared in the same way as in the preparation of the sample 108 except that an equimolar of each of a coupler component composed of C-7/C-30 (molar ratio: 3/1), a coupler component composed of C-7/C-10 (molar ratio: 2/1) and a coupler component composed of C-10 was used in place of the coupler C-30.

### Samples 112 to 113

Each of samples 112 to 113 was prepared in the same way as in the preparation of the sample 111 except that an equimolar amount of each of colored coupler 13 and 28 was used in place of colored coupler used for the sample 111.

These samples were subjected to white exposure for sensitometry and then to the color development as shown below. Cyan density and yellow density of the developed samples were measured. Relative sensitivity was determined as the logarithm of the reciprocal of the exposure amount giving a cyan density of (Fog + 0.2). Color turbidity was determined by the yellow density at a density giving a cyan density of 1.0.

Development was carried out at 38°C under the following conditions.

Each processing solution used in each stage had the following composition.

### Color Developing Solution

### Bleaching Solution

### Fixing Solution

### Stabilizing Solution

It is apparent from Table 1 that the samples obtained by using the couplers of the present invention had low color turbidity without reducing sensitivity and were superior from the viewpoint of color reproducibility in comparison with the samples without couplers of the present invention.

### EXAMPLE 2

The surface of a cellulose triacetate film support having an undercoat layer applied thereto was multi-coated with the following layers having the following compositions to prepare a multi-layer color photographic material as a sample 201.

### Compositions of Layers

The values for each component are coating weights in terms of g/m². The amount of silver halide is the coating weight in terms of silver. The amounts of sensitizing dyes are represented by moles per mol of silver halide in the same layer.

### Sample 201

### First Layer: Antihalation Layer

### Second Layer: Interlayer

### Third Layer: First Red-sensitive Emulsion Layer

### Fourth Layer: Second Red-sensitive Emulsion Layer

### Fifth Layer: Third Red-sensitive Emulsion Layer

### Sixth Layer: Interlayer

### Seventh Layer: First Green-sensitive Emulsion Layer

### Eighth Layer: Second Green-sensitive Emulsion Layer

### Ninth Layer: Third Green-sensitive Emulsion Layer

### Tenth Layer: Yellow Filter Layer

### Eleventh Layer: First Blue-sensitive Emulsion Layer

### Twelfth Layer: Second Blue-sensitive Emulsion Layer

### Thirteenth Layer: Third Blue-sensitive Emulsion Layer

### Fourtheenth Layer: First Protective Layer

### Fifteenth Layer: Second Protective Layer

In addition to the above-described ingredients, a hardening agent H-1 for gelatin and surfactant were added to each layer.

### Sample 202

A sample 202 was prepared in the same way as in the preparation of the sample 201 except that an equimolar amount of the coupler (3) of the present invention was used in place of colored coupler EX-3 used in each of the fourth and fifth layers of the sample 201.

### Sample 203

A sample 203 was prepared in the same way as in the preparation of the sample 201 except that an equimolar amount of cyan coupler C-7 (preferably used in the present invention) was used in place of EX-2 used in each of the third, fourth and fifth layers of the sample 201 and an equimolar amount of cyan coupler C-34 was used in place of EX-4 used in the fifth layer of the sample 201.

### Samples 204 to 208

Each of samples 204 to 208 was prepared in the same way as in the preparation of the sample 203 except that an equimolar amount of each of the couplers (1), (2), (3), (4) and (24) of the present invention was used in place of colored coupler EX-3 used in each of the fourth and fifth layers of the sample 203.

These samples were subjected to imagewise red exposure and then to the following color development. Relative sensitivity and color turbidity were then determined. Relative sensitivity was a relative value which was determined by the logarithm of the reciprocal of exposure amount giving a cyan density of (Fog + 0.2) when the sensitivity of the sample 201 was referred to as 0. Color turbidity was the value obtained by subtracting the fogged yellow density from the yellow density at a density giving a cyan density of (Fog + 1.5).

After the processed samples were left to stand at 80°C and 70% RH for two days, cyan density was re-measured. Cyan density at a point of an initial density of 1.00 was referred to as a density after forced deterioration.

The results are shown in Table 2.

Color development was carried out at 38°C under the following conditions by using an automatic processor.
- Color development: 3 min 15 sec
- Bleaching: 1 min
- Bleaching-fixing: 3 min 15 sec
- Rinse with water (1): 40 sec
- Rinse with water (2): 1 min
- Stabilization: 40 sec
- Drying (50°C): 1 min 15 sec

In the above processing stages, rinse (1) and (2) were a countercurrent rinse system from (2) to (1). Each processing solution had the following composition.

The replenishment rate of each processing solution was such that the replenishment rate of color developing solution was 1200 ml per m² of the color photographic material and that of each of other processing solutions including rinse was 800 ml. The amount of the processing solution came over from the previous-bath to the rinse stage was 50 ml per m² of the color photographic material.

### Color Developing Solution

### Bleaching Solution

Solution and replenischer were the same.

### Bleaching-fixing Solution

Solution and replenisher were the same.

### Rinsing Water

Tap water containing calcium ion (32 mg/ℓ) and magnesium ion (7.3 mg/ℓ) was passed through a column packed with an H type strongly acidic cation exchange resin and an OH type strongly basic anion exchange resin to reduce calcium ion to 1.2 mg/ℓ and magnesium ion to 0.4 mg/ℓ. Sodium isocyanurate dichloride in amount of 20 mg/ℓ was then added to the treated water.

### Stabilizing Solution

Solution and replenisher were the same.

### Drying

Drying temperature was 50°C.

It is apparent from Table 2 that the samples of the present invention exhibited low color turbidity and scarcely reduced the density of the cyan dye image under forced deterioration conditions.

### EXAMPLE 3

Each of samples 301 to 303 was prepared in the same way as in the preparation of the sample 201 except that each of the couplers (24), (26) and (28) of the present invention in an amount of 0.008 g/m² was added to the three layers of the seventh, eighth and ninth layers of the sample 201.

These samples were subjected to imagewise green exposure and then color-developed in the same manner as in Example 2. The density of each of the developed samples was measured. Color turbidity was determined as a value obtained by subtracting the fogged yellow density from the yellow density at a density giving a magenta density of (Fog + 1.0). The results are shown in Table 3. It is apparent from Table 3 that the samples containing the couplers of the present invention reduced color turbidity and provided excellent color reproducibility.

### EXAMPLE 4

The surface of a cellulose triacetate film support having an undercoat applied thereto was coated with the following layers having the following compositions to prepare a multi-layer color photographic material as a sample 401.

### Compositions of Layers

### First Layer: Antihalation Layer

### Second Layer: Low-sensitivity Red-sensitive Emulsion Layer

### Third Layer: Medium-sensitivity Red-sensitive Emulsion Layer

### Fourth Layer: High-sensitivity Red-sensitive Emulsion Layer

### Fifth Layer: Interlayer

### Sixth Layer: Low-sensitivity Green-sensitive Emulsion Layer

### Seventh Layer: Medium-sensitivity Green-sensitive Emulsion Layer

### Eight Layer: High-sensitivity Green-sensitive Emulsion Layer

### Ninth Layer: Interlayer

### Tenth Layer: Donor Layer Having Multilayer Effect on Red-sensitive Layer

### Eleventh Layer: Yellow Filter Layer

### Twelfth Layer: Low-sensitivity Blue-sensitive Emulsion Layer

### Thirteenth Layer: Interlayer

### Fourteenth Layer: High-sensitivity Blue-sensitive Emulsion Layer

### Fifteenth Layer: First Protective Layer

### Sixteenth Layer: Second Protective Layer

In addition to the above-described ingredients, stabilizer Cpd-3 (0.07 g/m²) for emulsions and surfactants W-1 (0.006 g/m²), W-2 (0.33 g/m²) and W-3 (0.10 g/m²) as coating aid or emulsifying dispersant were added to each layer.

Further, 1,2-benzisothiazoline-3-one, 2-phenoxyethanol and phenethyl alcohol were added to improve mildewproofness and antifungal properties.

### Samples 402 to 408

A sample 402 was prepared in the same way as in the preparation of the sample 401 except that comparative colored coupler R-1 in an amount of 0.020 g/m², 0.025 g/m² and 0.050 g/m² was added to the first layer, the second layer and the fourth layer of the sample 401, respectively.

Each of samples 403 to 408 was prepared in the same way as in the preparation of the sample 402 except that an equal weight of each of colored couplers indicated in Table 4 was used in place of colored coupler R-1.

These samples were subjected to imagewise red exposure and then color-developed in the same manner as in Example 1. Relative sensitivity and color turbidity were determined in the same manner as in Example 2.

It is apparent from Table 4 that the samples of the present invention were highly sensitive and reduced color turbidity.

The compounds used in Examples 1, 2, 3 and 4 were as follows:
U-1
U-2
U-3
U-4 (Suffixes of parenthesis show weight ratio)
U-5
EX-1
EX-2
EX-3 (Coupler 4 of JP-A-61-273543)
EX-4
EX-5
EX-6 (Suffixes of parenthesis show weight ratio) Average M.W. 30,000
EX-7
EX-8 (a mixture of compounds substituted at the 5- or 6-position)
EX-9
EX-10
EX-11
EX-12
S-1
S-2
HBS-1 Tricresyl phosphate
HBS-2 Dibutyl phthalate
HBS-3 Tri(n-hexyl)phosphate
EX-13
EX-14
EX-15
EX-16 (a mixture of compounds substituted at the 5- or 6-position)
EX-17 (a mixture of compounds substituted at the 5- or 6-position)
EX-18 (a mixture of compounds substituted at the 5- or 6-position)
HBS-11
H-1

Sensitizing dye
I
II
III
IV
V
VI
VII
VIII
IX
X R-1 (C-15 of JP-A-61-221748) R-2 (C-17 of JP-A-61-221748)

Cpd-1
Cpd-2
Cpd-3
Cpd-4 (Suffixes of parenthesis show weight ratio)
Cpd-5
Cpd-6
Cpd-7
Cpd-8

F-1
F-2
W-1
W-2
W-3
W-4

   C₈F₁₇SO₂N(C₃H₇)CH₂COOK

## Claims

1. A processing method comprising subjecting an image-wise exposed silver halide color photographic material comprising a support having thereon at least one light-sensitive silver halide emulsion layer and at least one colored coupler capable of releasing a water-soluble compound comprising a 6-hydroxy-2-pyridone-5-azo group by a coupling reaction with an oxidized aromatic primary amine developing agent to a wet color developing step and a step which uses a bath having bleaching ability.

2. The process as claimed in claim 1, wherein said colored coupler is represented by formula (I): wherein Cp represents a coupler moiety capable of being cleaved from -(T)_{ℓ} by a coupling reaction with an oxidized aromatic primary developing agent; T represents a timing group; ℓ is 0 or 1; X represents a divalent linking group bonded to (T)_{ℓ} through N, O or S; Y represents an arylene group or a divalent heterocyclic group; R₁ and R₂ each represents a hydrogen atom, a carboxyl group, a sulfo group, a cyano group, an alkyl group, a cycloalkyl group, an aryl group, a heterocyclic group, a carbamoyl group, a sulfamoyl group, a carbonamido group, a sulfonamido group or an alkylsulfonyl group; and R₃ represents a hydrogen atom, an alkyl group, a cycloalkyl group, an aryl group or a heterocyclic group, provided that at least one of R₁, R₂ and R₃ comprises a water-solubilizing group.

3. The process as claimed in claim 2, wherein said heterocyclic group represented by Y, R₁, R₂ or R₃ is a 3-membered to 8-membered substituted or unsubstituted heterocyclic group and containing at least one hetero-atom selected from the group consisting of N, O, S, P, Se and Te.

4. The process as claimed in claim 2, wherein said coupler moiety represented by Cp is represented by formulae (Cp-1), (Cp-2), (Cp-3), (Cp-4), (Cp-5), (Cp-6), (Cp-7), (Cp-8), (Cp-9) or (Cp-10): wherein the free bond indicates the position bonded to -(T)_{ℓ} in formula (I); R₅₁ represents R₄₁; R₅₂ and R₅₃ each represents R₄₂; R₅₄ represents R₄₁, R₄₁S-, R₄₃O-, or N≡C-; R₅₅ represents R₄₁; R₅₆ and R₅₇ each represents R₄₃, R₄₁S-, R₄₃O-, R₅₈ represents R₄₁; R₅₉ represents R₄₁, R₄₁O-, R₄₁S-, a halogen atom or d is 0 or an integer from 1 to 3; when d is 2 or 3, R₅₉ groups may be divalent groups which bond to each other to form a ring structure;
R₆₀ represents R₄₁; R₆₁ represents R₄₁; R₆₂ represents R₄₁, R₄₁CONH-, R₄₁OCONH-, R₄₁SO₂NH-, R₄₃O-, R₄₁S-, a halogen atom or R₆₃ represents R₄₁, R₄₁SO₂-, R₄₃OCO-, R₄₃O-SO₂-, a halogen atom, a nitro group, a cyano group or R₄₃CO-; and e is 0 or an integer of 1 to 4;
wherein R₄₁ represents a aliphatic group, an aromatic group or a heterocyclic group; R₄₂ represents an aromatic group or a heterocyclic group; and R₄₃, R₄₄ and R₄₅ each represents a hydrogen atom, an aliphatic group, an aromatic group or a heterocyclic group; and a bis type, telomer type and polymer type coupler moiety formed by bonding the coupler moieties at R₅₁, R₅₂; R₅₃; R₅₄, R₅₅, R₅₆, R₅₇, R₅₈, R₅₉, R₆₀, R₆₁, R₆₂ and R₆₃.

5. The process as claimed in claim 4, wherein said aliphatic hydrocarbon group aromatic group and heterocyclic group have at least one substituent selected from the group consisting of a halogen atom, R₄₇O-, R₄₆S-, R₄₆SO₂-, R₄₇OCO-, a group having the same meaning as R₄₆, R₄₆COO-, R₄₇OSO₂, a cyano group and a nitro group, whrein R₄₆ is an aliphatic group, an aromatic group or a heterocyclic group and R₄₇, R₄₈ and R₄₉ are each an aliphatic group, an aromatic group, a heterocyclic group or hydrogen atom.

6. The process as claimed in claim 4, wherein said coupler represented by Cp is a cyan coupler represented by formula (Cp-7) or (Cp-8).

7. The process as claimed in claim 2, wherein said timing group is selected from the group consisting of groups which utilize the cleavage reaction of hemiacetal, groups which undergo a cleavage reaction by utilizing an intermolecular nucleophilic substitution reaction, groups which undergo a cleavage reaction by utilizing an electron transfer reaction along a conjugated system, groups which utilize a cleavage reaction by the hydrolysis of an ester, groups which utilize a cleavage reaction of an imino-ketal, and a combination thereof.

8. The process as claimed in claim 2, wherein said timing group is represented by formulae (T-1), (T-2), (T-3), (T-4), (T-5), (T-6) or a combination thereof: wherein * represents the position where T is bonded to Cp in formula (I) and ** represents the position where T is bonded to X in formula (I); W represents oxygen, sulfur or R₁₁ and R₁₂ each represents a hydrogen atom, R₁₅, R₁₅CO-, R₁₅SO₂-, R₁₃ represents R₁₅, R₁₅CO-, R₁₅SO₂-, R₁₅ represents an aliphatic group, an aromatic group or a heterocyclic group; R₁₆ represents a hydrogen atom, an aliphatic group, an aromatic group or a heterocyclic group; R₁₁ and R₁₂ each may be a divalent group and bonds to each other to form a ring; and t is 1 or 2;
*-Nu-Link-E-** (T-2)
wherein * and ** are as defined in formula (T-1); Nu represents a nucleophilic group; E represents an electrophilic group capable of cleaving the bond marked ** by nucleophilic attack by Nu; and Link represents a linking group through which Nu and E are stearically positioned such that an intramolecular nucleophilic substitution reaction takes place; wherein * and **, W, R₁₁, R₁₂ and t are each as defined in formula (T-1), R₁₁ and R₁₂ may be bonded to form a benzene ring, and W and R₁₁ or R₁₂ may be bonded to form a benzene ring or a heterocyclic group; Z₁ and Z₂ each represents a carbon or nitrogen atom; x and y each is 0 or 1, provided that when Z₁ represents a carbon atom, x is 1, when Z₁ represents a nitrogen atom, x is 0, when Z₂ represents carbon, y is 1 and when Z₂ represents a nitrogen atom, y is 0; wherein *, **, and W are as defined in formula (T-1), and R₁₄ has the same definition as R₁₃ in formula (T-1).

9. The process as claimed in claim 8, wherein said timing group is represented by formulae (T-1), (T-2) or (T-3).

10. The process as claimed in claim 2, wherein X is a divalent group bonded to (T)1 through N, O or S.

11. The process as claimed in claim 2, wherein X is -O-, -S-, -OSO₂-, -OSO₂NH-, divalent heterocyclic group bonded to (T)_{ℓ} through N, or a bonding group which is a composite group derived from these groups and an alkylene group, a cycloalkylene group, an arylene group, a divalent hererocyclic group, CO-, -SO₂-, -COO-, -CONH-, -SO₂NH-, -SO₂O-, -NHCO-, NHSO₂-, -NHCONH-, -NHSO₂NH-, or -NHCOO-.

12. The process as claimed in claim 2, wherein X is represented by formula (II):
*-X₁-(L-X₂)ₘ-** (II)
wherein * represents the position where X₁ is bonded to (T)_{ℓ}; ** represents the position where X₂ is bonded to Y; X₁ represents -O- or -S-; L represents an alkylene group; X₂ represents a single bond, -O-, -S-, -CO-, -SO₂-, -SO₂NH-, -NHSO₂-, -SO₂O-, -OSO₂-, -NHSO₂NH-, -OSO₂NH- or -NHSO₂O-; and m is 0 or an integer of 1 to 3.

13. The process as claimed in claim 2, wherein said arylene group represented by Y is a substituted arylene group or a substituted heterocyclic group substituted with at least one of substituent selected from the group consisting of a halogen atom, a hydroxyl group, a nitro. group, a cyano group, an alkyl group, a cycloalkyl group, an aryl group, a carbonamido group, a sulfonamido group, an alkoxy group, an aryloxy group, an acyl group, a sulfonyl group, a carboxyl group, a sulfo group, a carbamoyl group, and a sulfamoyl group.

14. The process as claimed in claim 2, wherein said alkyl group, cycloalkyl group and heterocyclic group represented by R₁, R₂, or R₃ have at least one substituent selected from the group consisting of a halogen atom, a hydroxyl group, a carboxyl group, a sulfo group, a phosphono group, a phosphino group, a cyano group, an alkoxy group, an aryl group, an alkoxycarbonyl group, an amino group, an ammonium group, an acyl group, a carbonamido group, a sulfonamido group, a carbamoyl group, a sulfamoyl group and sulfonyl group.

15. The process as claimed in claim 2, wehrein said aryl group represented by R₁, R₂, or R₃ have at least one substituent selected from the group consisting of a halogen atom, a hydroxyl group, a carboxyl group, a sulfo group, a phosphono group, a phosphino group, a cyano group, an alkoxy group, an aryl group, an alkoxycarbonyl group, an amino group, an ammonium group, an acyl group, a carbonamido group, a sulfonamido group, a carbamoyl group, a sulfamoyl group, sulfonyl group, an alkyl group and a cycloalkyl group.

16. The process as claimed in claim 2, wherein said compound represented by formula (I) is contained in an amount of 1x10⁻⁶ to 3x10⁻³ mol/m².

17. The process as claimed in claim 2, wherein said compound represented by formula (I) is present in said light-sensitive silver halide emulsion layer.

18. The process as claimed in claim 17, wherein said light-sensitive silver halide emulsion layer contains an uncolored coupler.

19. The process as claimed in claim 17, wherein said uncolored coupler is a cyan coupler.

20. The process as claimed in claim 17, wherein said uncolored coupler is a naphthol cyan coupler.

21. The process as claimed in claim 17, wherein said uncolored coupler is a compound represented by formula (C): wherein R₁ represents -CONR₄R₅, -SO₂NR₄R₅, -NHCOR₄, -NHCOOR₆, -NHSO₂R₆, -NHCONR₄R₅ or -NHSO₂NR₄R₅; R₂ represents a halogen atom, a hydroxyl group, a carboxyl group, an amino group, a sulfo group, a cyano group, an alkyl group, an aryl group, a heterocyclic group, a carbonamido group, a sulfonamido group, a carbamoyl group, a sulfamoyl group, a ureido group, an acyl group, an acyloxy group, an alkoxy group, an aryloxy group, an alkylthio group, an arylthio group, an alkylsulfonyl group, an arylsulfonyl group, a sulfamoylamino group, an alkoxycarbonylamino group, a nitro group or an imido group; ℓ is 0 or an integer of 1 to 3; R₃ represents R₇(Y)ₘ-, wherein Y represents 〉NH, 〉CO or 〉SO₂, m is 0 or 1; and R₇ represents a hydrogen atom, an alkyl group containing 1 to 30 carbon atoms, an aryl group containing 6 to 30 carbon atoms, a heterocyclic group containing 2 to 30 carbon atoms, -COR₈, -OR₁₀, -CO₂R₁₀, -SO₂OR₁₀ or -SO₂R₁₀;
X represents a hydrogen atom or a group capable of being eliminated by a coupling reaction with an oxidized aromatic primary amine developing agent; R₄ and R₅ each represents a hydrogen atom, an alkyl group, an aryl group or a heterocyclic group; and R₆, R₈, R₉ and R₁₀ each represents an alkyl group, an aryl group or a heterocyclic group; two groups of R₂, R₂ and R₃, and R₃ and X may be bonded to each other to form a ring; R₄ and R₅, and R₈ and R₉ may be bonded to each other to form a heterocyclic ring containing at least one nitrogen atom; or a bis compound or a polymer may be formed through a group of divalence or higher at R₁, R₂, R₃ or X.

22. Use of a colored coupler capable of releasing a water-soluble compound comprising a 6-hydroxy-2-pyridone-5-azo group by a coupling reaction with an oxidized aromatic primary amine developing agent as defined in claims 1 to 15 for reducing color turbidity in a process according to claim 1.

## Patentansprüche

1. Verarbeitungsverfahren (Processing-Verfahren), umfassend das Unterwerfen eines bildweise belichteten farbphotografischen Silberhalogenidmaterials mit einem Träger und darauf mindestens einer lichtempfindlichen Silberhalogenid-Emulsionsschicht und mindestens einem farbigen Kuppler, der imstande ist, eine wasserlösliche Verbindung mit einer 6-Hydroxy-2-pyridon-5-azo-Gruppe durch eine Kupplungsreaktion mit einem oxidierten aromatischen, primären Amin-Entwicklungsmittel freizusetzen, einem Farb-Nassentwicklungsschritt und einem Schritt, der ein Bad mit Bleichfähigkeit verwendet.

2. Verfahren gemäss Anspruch 1, bei dem der farbige Kuppler durch Formel (I) dargestellt wird: worin Cp eine Kupplereinheit darstellt, die von -(T)_{ℓ} durch eine Kupplungsreaktion mit einem oxidierten aromatischen, primären Entwicklungsmittel abgespalten werden kann; T eine Timing-Gruppe darstellt; ℓ 0 oder 1 ist; X eine zweiwertige verbindende Gruppe, die an -(T)_{ℓ} durch N, O oder S gebunden ist, darstellt; Y eine Arylengruppe oder eine zweiwertige heterocyclische Gruppe darstellt; R₁ und R₂ jeweils ein Wasserstoffatom, eine Carboxylgruppe, eine Sulfogruppe, eine Cyanogruppe, eine Alkylgruppe, eine Cycloalkylgruppe, eine Arylgruppe, eine heterocyclische Gruppe, eine Carbamoylgruppe, eine Sulfamoylgruppe, eine Carbonamidogruppe, eine Sulfonamidogruppe oder eine Alkylsulfonylgruppe darstellen; und R₃ ein Wasserstoffatom, eine Alkylgruppe, eine Cycloalkylgruppe, eine Arylgruppe oder eine heterocyclische Gruppe darstellt, mit der Massgabe, dass mindestens eine Gruppe aus R₁, R₂ und R₃ eine wasser-solubilisierende Gruppe umfasst.

3. Verfahren gemäss Anspruch 2, worin die durch Y, R₁, R₂ oder R₃ dargestellte heterocyclische Gruppe eine 3- bis 8-gliedrige substituierte oder unsubstituierte heterocyclische Gruppe ist, die mindestens ein Heteroatom, ausgewählt aus der Gruppe, bestehend aus N, O, S, P, Se und Te, enthält.

4. Verfahren gemäss Anspruch 2, worin die durch Cp dargestellte Kupplereinheit durch die Formeln (Cp-1), (Cp-2), (Cp-3), (Cp-4), (Cp-5), (Cp-6), (Cp-7), (Cp-8), (Cp-9) oder (Cp-10) dargestellt wird: worin die freie Bindung die Position angibt, die an -(T)_{ℓ} in Formel (I) gebunden ist; R₅₁ R₄₁ darstellt; R₅₂ und R₅₃ jeweils R₄₂ darstellen; R₅₄ darstellt: R₄₁, R₄₁S-, R₄₃O-, oder N≡-C-; R₅₅ R₄₁ darstellt;
R₅₆ und R₅₇ jeweils darstellen: R₄₃, R₄₁S-, R₄₃O-, R₅₈ R₄₁ darstellt; R₅₉ darstellt: R₄₁, R₄₁O-, R₄₁S-, ein Halogenatom oder d 0 oder eine ganze Zahl von 1 bis 3 ist; wenn d 2 oder 3 ist, die R₅₉-Gruppen zweiwertige Gruppen sein können, die miteinander unter Bildung einer Ringstruktur verbunden sind; R₆₀ R₄₁ darstellt; R₆₁ R₄₁ darstellt; R₆₂ darstellt: R₄₁, R₄₁CONH-, R₄₁OCONH-, R₄₁SO₂NH-, R₄₃O-, R₄₁S-, ein Halogenatom oder R₆₃ darstellt: R₄₁, R₄₁SO₂-, R₄₃OCO-, R₄₃O-SO₂-, ein Halogenatom, eine Nitrogruppe, eine Cyanogruppe oder R₄₃CO-; und e 0 oder eine ganze Zahl von 1 bis 4 ist;
wobei R₄₁ eine aliphatische Gruppe, eine aromatische Gruppe oder eine heterocyclische Gruppe darstellt; R₄₂ eine aromatische Gruppe oder eine heterocyclische Gruppe darstellt; und R₄₃, R₄₄ und R₄₅ jeweils ein Wasserstoffatom, eine aliphatische Gruppe, eine aromatische Gruppe oder eine heterocyclische Gruppe darstellen; und eine Kupplereinheit vom Bistyp, Telomertyp und Polymertyp, gebildet durch Verbinden der Kupplereinheiten bei R₅₁, R₅₂, R₅₃, R₅₄, R₅₅, R₅₆, R₅₇, R₅₈, R₅₉, R₆₀, R₆₁, R₆₂ und R₆₃.

5. Verfahren gemäss Anspruch 4, wobei die aliphatische Kohlenwasserstoffgruppe, die aromatische Gruppe und die heterocyclische Gruppe mindestens einen Substituenten haben, der ausgewählt ist aus der Gruppe, bestehend aus einem Halogenatom, R₄₇O-, R₄₆S-, R₄₆SO₂- R₄₇OCO-, eine Gruppe mit derselben Bedeutung wie R₄₆, R₄₆COO-, R₄₇OSO₂, einer Cyanogruppe und einer Nitrogruppe, wobei R₄₆ eine aliphatische Gruppe, eine aromatische Gruppe oder eine heterocyclische Gruppe ist, und R₄₇, R₄₈ und R₄₉ jeweils eine aliphatische Gruppe, eine aromatische Gruppe, eine heterocyclische Gruppe oder ein Wasserstoffatom sind.

6. Verfahren gemäss Anspruch 4, worin der durch Cp dargestellte Kuppler ein Cyankuppler ist, der durch die Formeln (Cp-7) oder (Cp-8) dargestellt wird.

7. Verfahren gemäss Anspruch 2, worin die Timing-Gruppe ausgewählt ist aus der Gruppe, bestehend aus Gruppen, die die Spaltungsreaktion eines Hemiacetals nutzen, Gruppen, die eine Spaltungsreaktion durch Nutzung einer intramolekularen nukleophilen Substitutionsreaktion erfahren, Gruppen, die eine Spaltungsreaktion durch Nutzung einer Elektronentransferreaktion entlang eines konjugierten Systems erfahren, Gruppen, die eine Spaltungsreaktion durch die Hydrolyse eines Esters nutzen, Gruppen, die eine Spaltungsreaktion eines Iminoketals nutzen, und einer Kombination davon.

8. Verfahren gemäss Anspruch 2, worin die Timing-Gruppe durch die Formeln (T-1), (T-2), (T-3), (T-4), (T-5), (T-6) oder einer Kombination davon dargestellt wird: worin * die Position darstellt, in der T an Cp in Formel (I) gebunden ist, und ** die Position darstellt, in der T mit X in der Formel (I) gebunden ist; W Sauerstoff, Schwefel oder darstellt; R₁₁ und R₁₂ jeweils ein Wasserstoffatom, R₁₅, R₁₅CO-, R₁₅SO₂-, darstellen; R₁₃ R₁₅, R₁₅CO-, R₁₅SO₂, darstellt; R₁₅ eine aliphatische Gruppe, eine aromatische Gruppe oder eine heterocyclische Gruppe darstellt; R₁₆ ein Wasserstoffatom, eine aliphatische Gruppe, eine aromatische Gruppe oder eine heterocyclische Gruppe darstellt; R₁₁ und R₁₂ beide eine zweiwertige Gruppe sein können und miteinander unter Bildung eines Rings verbunden sind; und t 1 oder 2 ist;
*-Nu-Link-E-** (T-2)
worin * und ** wie in Formel (T-1) definiert sind; Nu eine nukleophile Gruppe darstellt; E eine elektrophile Gruppe darstellt, die imstande ist, die durch ** markierte Bindung bei nukleophiler Attacke durch Nu zu spalten; und Link eine verbindende Gruppe darstellt, durch die Nu und E sterisch so angeordnet werden, dass eine intramolekulare nukleophile Substitutionsreaktion stattfindet; worin * und **, W, R₁₁, R₁₂ und t jeweils wie in Formel (T-1) definiert sind, R₁₁ und R₁₂ unter Bildung eines Benzolrings verbunden sein können und W und R₁₁ oder R₁₂ unter Bildung eines Benzolrings oder einer heterocyclischen Gruppe verbunden sein können; Z₁ und Z₂ jeweils ein Kohlenstoffatom oder ein Stickstoffatom darstellen; x und y jeweils 0 oder 1 sind, mit der Massgabe, dass, wenn Z₁ ein Kohlenstoffatom darstellt, x 1 ist, wenn Z₁ ein Stickstoffatom darstellt, x 0 ist; wenn Z₂ Kohlenstoff ist, y 1 ist, und wenn Z₂ ein Stickstoffatom ist, y 0 ist; worin *, ** und W wie in Formel (T-1) definiert sind und R₁₄ dieselbe Definition wie R₁₃ in Formel (T-1) hat.

9. Verfahren gemäss Anspruch 8, worin die Timing-Gruppe durch die Formeln (T-1), (T-2) oder (T-3) dargestellt wird.

10. Verfahren gemäss Anspruch 2, worin X eine zweiwertige Gruppe ist, die an (T)_{ℓ} durch N, O oder S gebunden ist.

11. Verfahren gemäss Anspruch 2, worin X ist: -O- -S-, -OSO₂-, -OSO₂NH-, eine zweiwertige heterocyclische Gruppe, die an (T)_{ℓ} durch N gebunden ist, oder eine Bindungsgruppe, die eine zusammengesetzte Gruppe aus diesen Gruppen und einer Alkylengruppe, einer Cycloalkylengruppe, einer Arylengruppe, einer zweiwertigen heterocyclischen Gruppe, -CO-, -SO₂-, -COO-, -CONH-, -SO₂NH-, -SO₂O-, -NHCO-, -NHSO₂-, -NHCONH-, -NHSO₂NH- oder -NHCOO- ist.

12. Verfahren gemäss Anspruch 2, worin X durch Formel (II) dargestellt wird:
*-X₁-(L-X₂)ₘ-** (II)
worin * die Position darstellt, in der X₁ an (T)_{ℓ} gebunden ist; ** die Position darstellt, in der X₂ an Y gebunden ist; X₁ -O- oder -S- darstellt; L eine Alkylengruppe darstellt; X₂ eine Einfachbindung, -O-, -S-, -CO-, SO₂-, -SO₂NH-, -NHSO₂-, -SO₂O-, -OSO₂-, -NHSO₂NH-, -OSO₂NH- oder -NHSO₂O- ist; und m 0 oder eine ganze Zahl von 1 bis 3 ist.

13. Verfahren gemäss Anspruch 2, worin die durch Y dargestellte Arylengruppe eine substituierte Arylengruppe oder eine substituierte heterocyclische Gruppe ist, die mit mindestens einem Substituenten substituiert ist, der ausgewählt wird aus der Gruppe, bestehend aus einem Halogenatom, einer Hydroxylgruppe, einer Nitrogruppe, einer Cyanogruppe, einer Alkylgruppe, einer Cycloalkylgruppe, einer Arylgruppe, einer Carbonamidogruppe, einer Sulfonamidogruppe, einer Alkoxygruppe, einer Aryloxygruppe, einer Acylgruppe, einer Sulfonylgruppe, einer Carboxylgruppe, einer Sulfogruppe, einer Carbamoylgruppe und einer Sulfamoylgruppe.

14. Verfahren gemäss Anspruch 2, worin die durch R₁, R₂ oder R₃ dargestellten Alkylgruppen, Cycloalkylgruppen und heterocyclischen Gruppen mindestens einen Substituenten haben, der ausgewählt ist aus der Gruppe, bestehend aus einem Halogenatom, einer Hydroxylgruppe, einer Carboxylgruppe, einer Sulfogruppe, einer Phosphonogruppe, einer Phosphinogruppe, einer Cyanogruppe, einer Alkoxygruppe, einer Arylgruppe, einer Alkoxycarbonylgruppe, einer Aminogruppe, einer Ammoniumgruppe, einer Acylgruppe, einer Carbonamidogruppe, einer Sulfonamidogruppe, einer Carbamoylgruppe, einer Sulfamoylgruppe und einer Sulfonylgruppe.

15. Verfahren gemäss Anspruch 2, worin die durch R₁, R₂ oder R₃ dargestellte Arylgruppe mindestens einen Substituenten hat, der ausgewählt ist aus der Gruppe, bestehend aus einem Halogenatom, einer Hydroxylgruppe, einer Carboxylgruppe, einer Sulfogruppe, einer Phosphonogruppe, einer Phosphinogruppe, einer Cyanogruppe, einer Alkoxygruppe, einer Arylgruppe, einer Alkoxycarbonylgruppe, einer Aminogruppe, einer Ammoniumgruppe, einer Acylgruppe, einer Carbonamidogruppe, einer Sulfonamidogruppe, einer Carbamoylgruppe, einer Sulfamoylgruppe, einer Sulfonylgruppe, einer Alkylgruppe und einer Cycloalkylgruppe.

16. Verfahren gemäss Anspruch 2, wobei die durch Formel (I) dargestellte Verbindung in einer Menge von 1 x 10⁻⁶ bis 3 x 10⁻³ Mol/m² enthalten ist.

17. Verfahren gemäss Anspruch 2, worin die durch Formel (I) dargestellte Verbindung in der genannten lichtempfindlichen Silberhalogenid-Emulsionsschicht vorliegt.

18. Verfahren gemäss Anspruch 17, wobei die genannte lichtempfindliche Silberhalogenid-Emulsionsschicht einen farblosen Kuppler enthält.

19. Verfahren gemäss Anspruch 17, wobei der farblose Kuppler ein Cyankuppler ist.

20. Verfahren gemäss Anspruch 17, wobei der farblose Kuppler ein Naphthol-Cyankuppler ist.

21. Verfahren gemäss Anspruch 17, wobei der farblose Kuppler eine Verbindung ist, die durch Formel (C) dargestellt wird: worin R₁ -CONR₄R₅, -SO₂NR₄R₅, -NHCOR₄, -NHCOOR₆, -NHSO₂R₆, -NHCONR₄R₅ oder -NHSO₂NR₄R₅ darstellt; R₂ ein Halogenatom, eine Hydroxylgruppe, eine Carboxylgruppe, eine Aminogruppe, eine Sulfogruppe, eine Cyanogruppe, eine Alkylgruppe, eine Arylgruppe, eine heterocyclische Gruppe, eine Carbonamidogruppe, eine Sulfonamidogruppe, eine Carbamoylgruppe, eine Sulfamoylgruppe, eine Ureidogruppe, eine Acylgruppe, eine Acyloxygruppe, eine Alkoxygruppe, eine Aryloxygruppe, eine Alkylthiogruppe, eine Arylthiogruppe, eine Alkylsulfonylgruppe, eine Arylsulfonylgruppe, eine Sulfamoylaminogruppe, eine Alkoxycarbonylaminogruppe, eine Nitrogruppe oder eine Imidogruppe darstellt; ℓ 0 oder eine ganze Zahl von 1 bis 3 ist; R₃ R₇(Y)ₘ- darstellt, wobei Y 〉NH, 〉CO oder 〉SO₂ darstellt; m 0 oder 1 ist; und R₇ ein Wasserstoffatom, eine Alkylgruppe mit 1 bis 30 Kohlenstoffatomen, eine Arylgruppe mit 6 bis 30 Kohlenstoffatomen, eine heterocyclische Gruppe mit 2 bis 30 Kohlenstoffatomen, -COR₈, -OR₁₀, CO₂R₁₀, -SO₂OR₁₀ oder -SO₂R₁₀ darstellt; X ein Wasserstoffatom oder eine Gruppe darstellt, die durch eine Kupplungsreaktion mit einem oxidierten aromatischen, primären Amin-Entwicklungsmittel eliminiert werden kann; R₄ und R₅ jeweils ein Wasserstoffatom, eine Alkylgruppe, eine Arylgruppe oder eine heterocyclische Gruppe darstellen; und R₆, R₈, R₉ und R₁₀ jeweils eine Alkylgruppe, eine Arylgruppe oder eine heterocyclische Gruppe darstellen; zwei R₂-Gruppen, R₂ und R₃ und R₃ und X miteinander unter Bildung eines Rings verbunden sein können; R₄ und R₅, und R₈ und R₉ miteinander unter Bildung eines heterocyclischen Rings mit mindestens einem Stickstoffatom verbunden sein können; oder eine Bis-Verbindung oder ein Polymer durch eine Gruppe mit zwei oder mehr Valenzen bei R₁, R₂, R₃ oder X gebildet werden kann.

22. Verwendung eins farbigen Kupplers, der eine wasserlösliche Verbindung mit einer 6-Hydroxy-2-pyridon-5-azo-Gruppe durch eine Kupplungsreaktion mit einem oxidierten aromatischen, primären Amin-Entwicklungsmittel freisetzen kann, wie definiert in den Ansprüchen 1 bis 15, zur Verringerung der Farbtrübung in einem Verfahren gemäss Anspruch 1.

## Revendications

1. Procédé de traitement consistant à faire subir à un matériau photographique couleur à base d'halogénure d'argent exposé suivant la forme d'une image comprenant un support portant au moins une couche d'émulsion d'halogénure d'argent sensible à la lumière et au moins un agent de couplage coloré capable de libérer un composé soluble dans l'eau comprenant un groupe 6-hydroxy-2-pyridone-5-azo par une réaction de couplage avec un révélateur de type amine primaire aromatique oxydée, une étape de développement couleur par voie humide et une étape qui utilise un bain présentant des propriétés de blanchiment.

2. Procédé selon la revendication 1, dans lequel l'agent de couplage coloré répond à la formule (I) : dans laquelle Cp représente un reste d'agent de couplage pouvant être séparé de -(T)_{ℓ} par une réaction de couplage avec un révélateur de type amine aromatique primaire oxydée; T représente un groupe de réglage; ℓ est égal à O ou à 1; X représente un groupe de liaison divalent lié à (T)_{ℓ} par l'intermédiaire de N, O ou S; Y représente un groupe arylène ou un groupe hétérocyclique divalent; R₁ et R₂ représentent chacun un atome d'hydrogène, un groupe carboxy, un groupe sulfo, un groupe cyano, un groupe alkyle, un groupe cycloalkyle un groupe aryle, un groupe hétérocyclique, un groupe carbamoyle, un groupe sulfamoyle, un groupe carbonamido, un groupe sulfonamido ou un groupe alkylsulfonyle; et R₃ représente un atome d'hydrogène, un groupe alkyle, un groupe cycloalkyle, un groupe aryle ou un groupe hétérocyclique, à condition qu'au moins un des groupes R₁, R₂ et R₃ comprenne un groupe permettant la solubilité dans l'eau.

3. Procédé selon la revendication 2, dans lequel le groupe hétérocyclique représenté par Y, R₁, R₂ ou R₃ est un groupe hétérocyclique à 3 à 8 chaînons, substitué ou non et contenant au moins un hétéro-atome choisi dans le groupe constitué de N, O, S, P, Se et Te.

4. Procédé selon la revendication 2, dans lequel le reste d'agent de couplage représenté par Cp répond aux formules (Cp-1), (Cp-2), (Cp-3), (Cp-4), (Cp-5), (Cp-6), (Cp-7), (Cp-8), (Cp-9) ou (Cp-10) : dans lesquelles la liaison libre indique la position liée à -(T)_{ℓ}, dans la formule (I); R₅₁ représente R₄₁; R₅₂ et R₅₃ représentent chacun R₄₂; R₅₄ représente R₄₁, R₄₁S-, R₄₃O-, ou N≡C-; R₅₅ représente R₄₁; R₅₆ et R₅₇ représentent chacun R₄₃, R₄₁S-, R₄₃O-, ou R₅₈ représente R₄₁; R₅₉ représente R₄₁, R₄₁O-, R₄₁S-, un atome d'halogène ou d est égal à 0 ou à un nombre entier compris entre 1 et 3; lorsque d est égal à 2 ou à 3, les groupes R₅₉ peuvent être des groupes divalents liés les uns aux autres pour former une structure cyclique; R₆₀ représente R₄₁; R₆₁ représente R₄₁; R₆₂ représente R₄₁, R₄₁CONH-, R₄₁OCONH-, R₄₁SO₂NH-, R₄₃O-, R₄₁S-, un atome d'halogène ou R₆₃ représente R₄₁, R₄₁SO₂-, R₄₃OCO-, R₄₃O-SO₂-, un atome d'halogène, un groupe nitro, un groupe cyano ou R₄₃CO-; et e est égal à 0 ou à un nombre entier compris entre 1 et 4;
sachant que R₄₁ représente un groupe aliphatique, un groupe aromatique ou un groupe hétérocyclique; R₄₂ représente un groupe aromatique ou un groupe hétérocyclique; et R₄₃, R₄₄ et R₄₅ représentent chacun un atome d'hydrogène, un groupe aliphatique, un groupe aromatique ou un groupe hétérocyclique; et est un reste d'agent de couplage de type bis, de type télomère et de type polymère formé par liaison des restes d'agent de couplage en R₅₁, R₅₂, R₅₃, R₅₄, R₅₅, R₅₆, R₅₇, R₅₈, R₅₉, R₆₀, R₆₁, R₆₂ et R₆₃.

5. Procédé selon la revendication 4, dans lequel le groupe hydrocarboné aliphatique, le groupe aromatique et le groupe hétérocyclique ont au moins un substituant choisi dans le groupe constitué d'un atome d'halogène, R₄₇O-, R₄₆S-, R₄₆SO₂-, R₄₇OCO-, un groupe ayant le même sens que R₄₆, R₄₆COO-, R₄₇OSO₂, un groupe cyano et un groupe nitro, sachant que R₄₆ représente un groupe aliphatique, un groupe aromatique ou un groupe hétérocyclique et R₄₇, R₄₈ et R₄₉ représentent chacun un groupe aliphatique, un groupe aromatique, un groupe hétérocyclique ou un atome d'hydrogène.

6. Procédé selon la revendication 4, dans lequel le reste d'agent de couplage représenté par Cp est un reste d'agent de couplage cyan représenté par la formule (Cp-7) ou (Cp-8).

7. Procédé selon la revendication 2, dans lequel le groupe de réglage est choisi dans le groupe constitué de groupes qui utilisent la réaction de clivage d'un hémiacétal, de groupes qui subissent une réaction de clivage en utilisant une réaction de substitution nucléophile intermoléculaire, de groupes qui subissent une réaction de clivage en utilisant une réaction de transfert d'électron le long d'un système conjugué, de groupes qui utilisent une réaction de clivage par hydrolyse d'un ester, de groupes qui utilisent une réaction de clivage d'un imino-cétal, et une combinaison de ceux-ci.

8. Procédé selon la revendication 2, dans lequel le groupe de réglage est représenté par les formules (T-1), (T-2), (T-3), (T-4), (T-5), (T-6) ou une combinaison de celles-ci : dans laquelle * représente la position où T est lié à Cp dans la formule (I) et ** représente la position où T est lié à X dans la formule (I); W représente l'oxygène, le soufre ou R₁₁ et R₁₂ représentent chacun un atome d'hydrogène, R₁₅, R₁₅CO-, R₁₅SO₂-, R₁₃ représente R₁₅; R₁₅CO-, R₁₅SO₂-, R₁₅ représente un groupe aliphatique, un groupe aromatique ou un groupe hétérocyclique; R₁₆ représente un atome d'hydrogène, un groupe aliphatique, un groupe aromatique ou un groupe hétérocyclique; R₁₁ et R₁₂ peuvent chacun représenter un groupe divalent et être liés entre eux pour former un cycle; et t est égal à 1 ou à 2;
*-Nu-Link-E-** (T-2)
dans laquelle * et ** sont tels que définis pour la formule (T-1); Nu représente un groupe nucléophile; E représente un groupe électrophile capable de casser la liaison marquée ** par attaque nucléophile par Nu; et Link représente un groupe de liaison dans lequel Nu et E sont stériquement positionnés de façon à ce qu'une réaction de substitution nucléophile intramoléculaire ait lieu; dans laquelle * et **, W, R₁₁, R₁₂ et t sont chacun tels que définis pour la formule (T-1), R₁₁ et R₁₂ peuvent être liés pour former un cycle benzène, et W et R₁₁ ou R₁₂ peuvent être liés pour former un cycle benzène ou un groupe hétérocyclique; Z₁ et Z₂ représentent chacun un atome de carbone ou d'azote; x et y sont chacun égaux à 0 ou à 1, à condition que lorsque Z₁ représente un atome de carbone, x soit égal à 1, lorsque Z₁ représente un atome d'azote, x soit égal à 0, lorsque Z₂ représente un atome de carbone, y soit égal à 1 et lorsque Z₂ représente un atome d'azote, y soit égal à 0; dans lequel *, **, et W sont tels que définis pour la formule (T-1), et R₁₄ est tel que défini pour R₁₃ dans la formule (T-1).

9. Procédé selon la revendication 8, dans lequel le groupe de réglage est représenté par les formules (T-1), (T-2) ou (T-3).

10. Procédé selon la revendication 2, dans lequel X représente un groupe divalent lié à (T)_{ℓ} par N, O ou S.

11. Procédé selon la revendication 2, dans lequel X représente -O-, -S-, -OSO₂ , -OSO₂NH-, un groupe hétérocyclique divalent lié à (T)_{ℓ} par N, ou un groupe de liaison qui est un groupe composite dérivé de ces groupes et d'un groupe alkylène, un groupe cycloalkylène, un groupe arylène, un groupe hétérocyclique divalent, -CO-, -SO₂-, -COO-, -CONH-, -SO₂NH-, -SO₂O-, -NHCO-, NHSO₂-, -NHCONH-, -NHSO₂NH- ou -NHCOO-.

12. Procédé selon la revendication 2, dans lequel X répond à la formule (II) :
*-X₁-(L-X₂)ₘ-** (II)
dans laquelle * représente la position où X₁ est lié à (T)_{ℓ}; ** représente la position où X₂ est lié à Y; X₁ représente -O- ou -S-; L représente un groupe alkylène; X₂ représente une simple liaison, -O-, -S-, -CO-, -SO₂-, -SO₂NH-, -NHSO₂-, -SO₂O-, -OSO₂-, -NHSO₂NH-, -OSO₂NH- ou -NHSO₂O-; et m est égal à 0 ou à un nombre entier de 1 à 3.

13. Procédé selon la revendication 2, dans lequel le groupe arylène représenté par Y est un groupe arylène substitué ou un groupe hétérocyclique substitué, substitué avec au moins un substituant choisi dans le groupe constitué par un atome d'halogène, un groupe hydroxy, un groupe nitro, un groupe cyano, un groupe alkyle, un groupe cycloalkyle, un groupe aryle, un groupe carbonamido, un groupe sulfonamido, un groupe alcoxy, un groupe aryloxy, un groupe acyle, un groupe sulfonyle, un groupe carboxy, un groupe sulfo, un groupe carbamoyle, et un groupe sulfamoyle.

14. Procédé selon la revendication 2, dans lequel le groupe alkyle, le groupe cycloalkyle et le groupe hétérocyclique représentés par R₁, R₂ ou R₃ ont au moins un substituant choisi dans le groupe constitué par un atome d'halogène, un groupe hydroxy, un groupe carboxy, un groupe sulfo, un groupe phosphono, un groupe phosphino, un groupe cyano, un groupe alcoxy, un groupe aryle, un groupe alcoxycarbonyle, un groupe amino, un groupe ammonium, un groupe acyle, un groupe carbonamido, un groupe sulfonamido, un groupe carbamoyle, un groupe sulfamoyle et un groupe sulfonyle.

15. Procédé selon la revendication 2, dans lequel le groupe aryle représenté par R₁, R₂ ou R₃ a au moins un substituant choisi dans le groupe constitué par un atome d'halogène, un groupe hydroxy, un groupe carboxy, un groupe sulfo, un groupe phosphono, un groupe phosphino, un groupe cyano, un groupe alcoxy, un groupe aryle, un groupe alcoxycarbonyle, un groupe amino, un groupe ammonium, un groupe acyle, un groupe carbonamido, un groupe sulfonamido, un groupe carbamoyle, un groupe sulfamoyle, un groupe sulfonyle, un groupe alkyle et un groupe cycloalkyle.

16. Procédé selon la revendication 2, dans lequel le composé représenté par la formule (I) est contenu en une quantité de 1x10⁻⁶ à 3x10⁻³ mole/m².

17. Procédé selon la revendication 2, dans lequel le composé représenté par la formule (I) est présent dans la couche d'émulsion d'halogénure d'argent sensible à la lumière.

18. Procédé selon la revendication 17, dans lequel la couche d'émulsion d'halogénure d'argent sensible à la lumière contient un agent de couplage non coloré.

19. Procédé selon la revendication 17, dans lequel l'agent de couplage non coloré est un agent de couplage cyan.

20. Procédé selon la revendication 17, dans lequel l'agent de couplage non coloré est un agent de couplage cyan dérivé de naphtol.

21. Procédé selon la revendication 17, dans lequel l'agent de couplage non coloré est un composé répondant à la formule (C) : dans laquelle R₁ représente -CONR₄R₅, -SO₂NR₄R₅, -NHCOR₄, NHCOOR₆, -NHSO₂R₆, -NHCONR₄R₅ ou -NHSO₂NR₄R₅; R₂ représente un atome d'halogène, un groupe hydroxy, un groupe carboxy, un groupe amino, un groupe sulfo, un groupe cyano, un groupe alkyle, un groupe aryle, un groupe hétérocyclique, un groupe carbonamido, un groupe sulfonamido, un groupe carbamoyle, un groupe sulfamoyle, un groupe uréido, un groupe acyle, un groupe acyloxy, un groupe alcoxy, un groupe aryloxy, un groupe alkylthio, un groupe arylthio, un groupe alkylsulfonyle, un groupe arylsulfonyle, un groupe sulfamoylamino, un groupe alcoxycarbonylamino, un groupe nitro ou un groupe imido; ℓ est égal à 0 ou à un nombre entier de 1 à 3; R₃ représente R₇(Y)ₘ-, sachant que Y représente 〉NH, 〉CO ou 〉SO₂, m est égal à 0 ou à 1; et R₇ représente un atome d'hydrogène, un groupe alkyle contenant 1 à 30 atomes de carbone, un groupe aryle contenant 6 à 30 atomes de carbone, un groupe hétérocyclique contenant 2 à 30 atomes de carbone, -COR₈, -OR₁₀, -CO₂R₁₀, -SO₂OR₁₀ ou -SO₂R₁₀;
X représente un atome d'hydrogène ou un groupe pouvant être éliminé par une réaction de couplage avec un révélateur de type amine aromatique primaire oxydée; R₄ et R₅ représentent chacun un atome d'hydrogène, un groupe alkyle, un groupe aryle ou un groupe hétérocyclique; et R₆, R₈, R₉ et R₁₀ représentent chacun un groupe alkyle, un groupe aryle ou un groupe hétérocyclique; deux groupes de R₂, R₂ et R₃, et R₃ et X peuvent être liés entre eux pour former un cycle; R₄ et R₅, et R₈ et R₉ peuvent être liés entre eux pour former un hétérocycle contenant au moins un atome d'azote; ou un composé bis ou un polymère peut être formé par un groupe divalent ou de valence supérieure en R₁, R₂, R₃ ou X.

22. Utilisation d'un agent de couplage coloré capable de libérer un composé soluble dans l'eau comprenant un groupe 6-hydroxy-2-pyridone-5-azo par une réaction de couplage avec un révélateur de type amine primaire aromatique oxydée tel que défini dans les revendications 1 à 15, pour réduire le trouble des couleurs dans un procédé selon la revendication 1.
